

June 10, 1969

C. H. DAWSON

3,449,146

INDUCTION METHOD OF ARMORING METAL ARTICLES

Filed May 16, 1967

Sheet 1 of 34



INVENTOR

*Chester H. Dawson*  
BY  
*A. J. Miller*  
ATTORNEY

June 10, 1969

C. H. DAWSON

3,449,146

INDUCTION METHOD OF ARMORING METAL ARTICLES

Filed May 16, 1967

Sheet 2 of 34



June 10, 1969

C. H. DAWSON

3,449,146

INDUCTION METHOD OF ARMORING METAL ARTICLES

Filed May 16, 1967

Sheet 3 of 34



June 10, 1969

C. H. DAWSON

3,449,146

INDUCTION METHOD OF ARMORING METAL ARTICLES

Filed May 16, 1967

Sheet 4 of 34



June 10, 1969

C. H. DAWSON

3,449,146

## INDUCTION METHOD OF ARMORING METAL ARTICLES

Filed May 16, 1967

Sheet 5 of 34



June 10, 1969

C. H. DAWSON

3,449,146

INDUCTION METHOD OF ARMORING METAL ARTICLES

Filed May 16, 1967

Sheet 6 of 34

Fig 21

SICKLE SECTION  
TO BE COATED  
WITHIN DOTTED  
AREA



Fig 18

BRUSH ASSEMBLY



Fig 22



Fig 19



Fig 17

HINGE AND SLIDE SECTION



June 10, 1969

C. H. DAWSON

3,449,146

INDUCTION METHOD OF ARMORING METAL ARTICLES

Filed May 16, 1967

Sheet 7 of 34

Fig 23

### ADHESIVE APPLICATOR CIRCUIT



"HINGE" REFERS TO CARRIER-PARALLELOGRAM-HINGE

MECHANICAL and ELECTRICAL ACTIONS FOLLOW IN SEQUENCE FROM START to RETURN to READY  
UNLESS HAND OPERATED STOP SWITCH IS TURNED OFF TO "FREEZE"  
ACTION AT ANY DESIRED PHASE FOR SERVICING OR OTHERWISE



June 10, 1969

C. H. DAWSON

3,449,146

## INDUCTION METHOD OF ARMORING METAL ARTICLES

Filed May 16, 1967

Sheet 9 of 34



June 10, 1969

C. H. DAWSON

3,449,146

## INDUCTION METHOD OF ARMORING METAL ARTICLES

Filed May 16, 1967

Sheet 10 of 34



June 10, 1969

C. H. DAWSON

3,449,146

INDUCTION METHOD OF ARMORING METAL ARTICLES

Filed May 16, 1967

Sheet // of 34

719 32  
SLIDE AND HINGE ACTION DIAGRAM

No. 4 MOVEMENT IS NOT A DEFINITE LINE SHAPE AT TOP BECAUSE CENTERS AT BOTTOM SHIFT CONCURRENTLY.



CENTERS POSITIONS AT END OF MOTIONS 2 and 3 IS DETERMINED BY SWEEP ADJUSTMENT SHOWN IN FIG 16 and FIG 19

June 10, 1969

C. H. DAWSON

3,449,146

INDUCTION METHOD OF ARMORING METAL ARTICLES

Filed May 16, 1967

Sheet 12 of 34

T10 33

### ADHESIVE APPLICATOR CIRCUIT



T10 34

### SEQUENCE OF ELECTRICAL AND MECHANICAL ACTIONS

WEIGHT OF PART, HELD BY OPERATOR, DEPRESSES START-FORWARD-MOTION SWITCH WHICH ACTIVATES SOLENOID VALVE TO ALLOW PRESSURE INTO "START" END OF CYLINDER. WITH THIS PRESSURE ON PISTON, PARALLEL-GRAM HINGE CARRIES BRUSH UP OUT OF PAN AND OVER ONTO PART. THE SWITCH CONTACT CARRIER WHICH IS FASTENED TO LOWER PIECE OF HINGE IS MOVED FORWARD AT THE SAME TIME TILL LOWER BUMPER PRESSES END-FORWARD-MOTION SWITCH.

END-FORWARD-MOTION SWITCH ACTIVATES RELAY TO CLOSE OTHER CIRCUIT AND IS HELD CLOSED BECAUSE SAID CLOSING KEEPS RELAY COIL ENERGIZED UNTIL END-REVERSE-MOTION-NORMALLY-CLOSED SWITCH IS OPENED; THUS DROPPING RELAY INTO OPPOSITE POSITION. SYSTEM IS THEN READY FOR A NEW COMPLETE CYCLE.

DURING THE ABOVE SEQUENCE THE MECHANICAL COMPONENTS HAVE RETURNED TO THE READY POSITION.

June 10, 1969

C. H. DAWSON

3,449,146

INDUCTION METHOD OF ARMORING METAL ARTICLES

Filed May 16, 1967

Sheet 13 of 34

FIG. 35

PARTS FEEDER AND FUSING MECHANISM CIRCUIT



June 10, 1969

C. H. DAWSON

3,449,146

INDUCTION METHOD OF ARMORING METAL ARTICLES

Filed May 16, 1967

Sheet 14 of 34

T10 36

COLD ROLLED (AS ROLLED)  
HOT ROLLED (PICKLED AND AGGREGATE BLASTED)  
CAST (PICKLED, AGGREGATE BLASTED OR TUMBLED)  
MILLED (AS MILLED)  
FORGED (AGGREGATE BLASTED OR TUMBLED)

BRUSH, SPRAY, DIP OR PRINT.

PASS THRU CURTAIN FALLING FROM MAGNETIC FEEDER OR  
VIBRATING MESH BEFORE ADHESIVE SETS.

HEATED UNDER INFLUENCE OF PROTECTIVE ATMOSPHERE OR  
HEATED RAPIDLY WITH OR WITHOUT ATMOSPHERE SUCH AS  
INDUCTION HEATING.

PARTS, WHERE PRACTICAL, AND OF SUITABLY ALLOYED BASE  
METAL MAY BE IMMEDIATELY (WHILE STILL ABOVE CRITICAL  
TEMPERATURE) QUENCHED IN PROPER BATH AND SUBSE-  
QUENTLY TEMPERED TO DESIRED TOUGHNESS.

WASHING IN HOT SODA SOLUTION AND WATER OR PLAIN HOT  
WATER TO EITHER OF WHICH A RUST INHIBITOR HAS BEEN  
ADDED, THEN WIRE BRUSHING OR TUMBLING.

June 10, 1969

C. H. DAWSON

3,449,146

INDUCTION METHOD OF ARMORING METAL ARTICLES

Filed May 16, 1967

Sheet 15 of 34



June 10, 1969

C. H. DAWSON

3,449,146

INDUCTION METHOD OF ARMORING METAL ARTICLES

Filed May 16, 1967

Sheet 16 of 34



June 10, 1969

C. H. DAWSON

3,449,146

INDUCTION METHOD OF ARMORING METAL ARTICLES

Filed May 16, 1967

Sheet 17 of 34

Fig 40



Fig 41



Fig 42A



Fig 42B



Fig 42C



June 10, 1969

C. H. DAWSON

3,449,146

## INDUCTION METHOD OF ARMORING METAL ARTICLES

Filed May 16, 1967

Sheet 18 of 34

43



June 10, 1969

C. H. DAWSON

3,449,146

INDUCTION METHOD OF ARMORING METAL ARTICLES

Filed May 16, 1967

Sheet 19 of 34



June 10, 1969

C. H. DAWSON

3,449,146

INDUCTION METHOD OF ARMORING METAL ARTICLES

Filed May 16, 1967

Sheet 20 of 34

Fig 45

46 L.



Fig 46



Fig 47



June 10, 1969

C. H. DAWSON

3,449,146

INDUCTION METHOD OF ARMORING METAL ARTICLES

Filed May 16, 1967

Sheet 21 of 34



June 10, 1969

C. H. DAWSON

3,449,146

INDUCTION METHOD OF ARMORING METAL ARTICLES

Filed May 16, 1967

Sheet 22 of 34



June 10, 1969

C. H. DAWSON

3,449,146

## INDUCTION METHOD OF ARMORING METAL ARTICLES

Filed May 16, 1967

Sheet 23 of 34



June 10, 1969

C. H. DAWSON

3,449,146

INDUCTION METHOD OF ARMORING METAL ARTICLES

Filed May 16, 1967

Sheet 24 of 34



June 10, 1969

C. H. DAWSON

3,449,146

INDUCTION METHOD OF ARMORING METAL ARTICLES

Filed May 16, 1967

Sheet 25 of 34



June 10, 1969

C. H. DAWSON

3,449,146

INDUCTION METHOD OF ARMORING METAL ARTICLES

Filed May 16, 1967

Sheet 26 of 34



June 10, 1969

C. H. DAWSON

3,449,146

INDUCTION METHOD OF ARMORING METAL ARTICLES

Filed May 16, 1967

Sheet 27 of 34

Fig 63



Fig 64



Fig 65



June 10, 1969

C. H. DAWSON

3,449,146

INDUCTION METHOD OF ARMORING METAL ARTICLES

Filed May 16, 1967

Sheet 28 of 34



June 10, 1969

C. H. DAWSON

3,449,146

## INDUCTION METHOD OF ARMORING METAL ARTICLES

Filed May 16, 1967

Sheet 29 of 34



June 10, 1969

C. H. DAWSON

3,449,146

INDUCTION METHOD OF ARMORING METAL ARTICLES

Filed May 16, 1967

Sheet 30 of 34



June 10, 1969

C. H. DAWSON

3,449,146

INDUCTION METHOD OF ARMORING METAL ARTICLES

Filed May 16, 1967

Sheet 31 of 34



June 10, 1969

C. H. DAWSON

3,449,146

INDUCTION METHOD OF ARMORING METAL ARTICLES

Filed May 16, 1967

Sheet 32 of 34



June 10, 1969

C. H. DAWSON

3,449,146

INDUCTION METHOD OF ARMORING METAL ARTICLES

Filed May 16, 1967

Sheet 33 of 34



June 10, 1969

C. H. DAWSON

3,449,146

INDUCTION METHOD OF ARMORING METAL ARTICLES

Filed May 16, 1967

Sheet 34 of 34



**1**

3,449,146

**INDUCTION METHOD OF ARMORING  
METAL ARTICLES**

Chester H. Dawson, Danbury, Conn., assignor to Remington Arms Company, Inc., Bridgeport, Conn., a corporation of Delaware

Continuation-in-part of application Ser. No. 177,558, Mar. 5, 1962. This application May 16, 1967, Ser. No. 638,998

The portion of the term of the patent subsequent to Mar. 6, 1979, has been disclaimed

Int. Cl. C23c 3/04, 13/02; B44d 1/092

U.S. Cl. 117—22

8 Claims

**ABSTRACT OF THE DISCLOSURE**

The improved method comprises the operations of applying to a surface of a selected area of the metallic base of a metal article (steel or ferrous tool) an organic adhesive film of temporary character having the property of adhesion, of decomposing while undergoing pyrolysis as an incident to the method and of a consistency such that it spreads evenly and with a substantially uniform thickness on said surface upon contact therewith; producing with a vibrating feeder a curtain of falling powdered hard refractory metallic armoring material comprising powdered hard refractory metallic matrix alloy, borax and diamond substitute particles; passing said metal article with said adhesive film thereon through said curtain of falling powdered material until sufficient armoring material adheres to the organic adhesive on said selected area to form a relatively thin armor layer reproducing the entire selected area and contour of the surface beneath the adhesive including any square corner; initiating heating by means of alternating electric power of extremely high frequency to concentrate intense heat on the selected area of the surface of the steel article; and only momentarily continuing the intense heat concentrated on the surface of said selected surface area whereupon the organic adhesive is subject to pyrolysis causing constituents to evaporate, burn and produce reducing gases and products of combustion and a carbonaceous residue from any residual constituents to protect the metal article, the matrix alloy and the diamond substitute particles against oxidation and decarburization and the borax is fused to a plastic condition having holding properties and whereupon there is a fusion at the sweating temperature of the metallic matrix alloy of the hard refractory armor coating and the surface of said metal article at the interface thereby effecting a fusion of said hard refractory metallic matrix alloy of the armor coating and said metallic surface of said metal article and a merging together in a self-conforming, unitary armor layer of substantially uniform thickness with diamond substitute particles tightly fused therein and with a fused borax coating enveloping the unitary armor layer.

**RELATED APPLICATIONS**

The present application is a continuation-in-part of my co-pending United States application Ser. No. 177,558, filed Mar. 5, 1962 (now abandoned), which in turn is a continuation-in-part of application Ser. No. 546,779, filed Nov. 14, 1955, which in turn was a continuation-in-part application of Ser. No. 379,100, filed Sept. 8, 1953 (now abandoned), and which latter application was a continuation-in-part of my parent application, Ser. No. 41,180, filed July 28, 1948 (now abandoned). U.S. Patents No. 3,023,490 and No. 3,024,128 issued on applications Ser. No. 548,915 and No. 546,779, respectively.

The present invention relates to the art of producing

**2**

improved armored metal articles with a thin hard film made in situ and conforming to the exact contour of the underlying surface and, more particularly, to an improved induction method of armoring a selected surface of a metal article with a thin, flat, hard surface of smooth and uniform character and of uniform thinness containing particles of a diamond substitute and conforming to the exact contour of the selected surface, and to means for carrying the method into practice.

It is an object of the present invention to provide an improved induction method of applying a hard-wearing layer to a selected surface of a metal article to provide a thin hard armor and means for carrying the method into practice.

Another object of the invention is to provide an improved induction method of armoring metal articles with a thin hard film made in situ and conforming to the exact contour of the underlying surface and to use the induction method to effect the fusion of the thin armor film to the metal article.

The invention also contemplates providing an improved induction method of armoring by using concentrated and intense inductive heat on a selected surface of a metal article in order to fuse thereto a thin hard coating of smooth and uniform character containing particles of a diamond substitute and conforming substantially to the exact contour of the selected surface.

It is a further object of the invention to provide an improved induction method of applying in situ a hard armor surface to a tool made of a ferrous metal by means of controlled inductive heat intense enough to effectively fuse the armor to the surface of the ferrous tool.

The invention further contemplates providing an improved induction method of applying a hard abrasive film to a selected area of a metal article which requires no subsequent grinding and which can be used in the as-produced condition.

It is another object of the invention to provide an improved induction method of forming a refractory hard coating of cutting character on a metal article which is relatively free from tendency to chip off or shear off during use.

Still another object of the invention is to provide an improved induction method of applying in situ to a selected area of a steel tool a hard protective layer by inductively heating said layer and by concentrating said inductive heat on said area whereby an armored steel tool is produced.

It is likewise within the contemplation of the invention to provide an improved induction method of armoring metal articles in situ with a refractory coating which is thin, which has a relatively smooth, hard surface when initially applied, and which can preserve and conform to square corners of the internal and external types.

It is also the purpose of the invention to provide an improved induction method of applying an abrasive coating to a metal article which can be more quickly, easily and inexpensively applied than by prior methods and which includes the utilization of inductive heat to effect substantially instantaneous fusion of the coating to the metal article.

Among the further objects of the present invention is the provision of an improved method of inductively fusing in situ to a metal article a hard coating, layer, skin, etc., which results in a substantial saving of materials over prior methods, which is particularly valuable for armoring tools, which involves an exact control of metal to be applied, which obtains a firm controlled penetration forming a tenacious bond between the face of the article and the hard coating, which permits the retention by diamond substitutes of their effectiveness even during and after heat

treatment, which enables coated tools to be heat treated without substantial loss of hardness of the hard bonded coating, and which maintains the hardness, the abrasiveness and the sharpness of the armor even in service and even when heated in use up to red heat.

Other objects and advantages of the invention will become obvious from the following description taken in conjunction with the drawings, in which:

FIG. 1 illustrates a flow sheet of the improved induction method carrying an embodiment of the invention into practice and showing various operations thereof;

FIGS. 2 to 12 are diagrammatic views of operations and parts involved in the flow sheet illustrated in FIG. 1;

FIG. 13 is a diagrammatic illustration of an electric circuit involved in the improved induction method together with the electrical work coil;

FIG. 14 depicts a perspective view, with parts broken away for purposes of clarity, of a machine capable of applying an adhesive layer to an article, such as the one illustrated in FIG. 21;

FIG. 15 depicts a perspective view of a part of the machine illustrated in FIG. 14 in order to show the part containing adhesive and the brush in contact with the article;

FIG. 16 illustrates a side elevation, partly in section, of a parallelogram hinge and slide used in the machine to move the brush assembly from a pan containing adhesive to the article to be coated;

FIG. 17 is a sectional view of the parallelogram hinge and slide shown in FIG. 16;

FIG. 18 shows a detailed view, partly in section, of an applicator brush assembly for the machine illustrated in FIG. 14;

FIG. 19 is a detailed view of bumper 1035 used in the machine;

FIG. 20 is an enlarged detailed view of the self-centering screws and associated nuts used in FIG. 17;

FIG. 21 is a plan view of an article of manufacture, such as a steel sickle blade, which is to be armored;

FIG. 22 is a side elevational view of FIG. 21;

FIG. 23 shows the adhesive applicator circuit;

FIG. 24 is a perspective view of an induction machine for effecting instantaneous fusing of the armor coating and bonding it to the surface of the article by means of inductive heat;

FIGS. 25 and 26 show top plan views, with parts broken away for purposes of clarity, of the machine illustrated in FIG. 24;

FIG. 27 is an enlarged fragmentary plan view of the electrical work coil of the induction machine showing the connection with a high frequency (H.F.) source of alternating electric power;

FIG. 28 depicts a fragmentary cross sectional view of the electrical work coil shown in FIG. 27;

FIG. 29 shows a fragmentary side view of the fixturing block and coolant connections;

FIG. 30 illustrates a fragmentary perspective view of a carriage used in the machine of FIG. 24;

FIG. 31 is a fragmentary cross sectional view showing "wedge" camming used in the carriage illustrated in FIG. 30;

FIG. 32 illustrates the slide and hinge action diagram;

FIG. 33 shows an adhesive applicator circuit;

FIG. 34 depicts a sequence of electrical and mechanical actions or operations;

FIG. 35 shows the feeder parts and fusing mechanism circuit;

FIG. 36 illustrates steps in the present improved induction armoring process;

FIG. 37 is a perspective view of the machine illustrated in FIGS. 24 to 26 for armoring the article of manufacture (sickle section) shown in FIGS. 21 and 22;

FIG. 38 shows a top plan fragmentary view of FIG. 37 to depict the sickle sections approaching the electrical work coil;

FIG. 39 illustrates a side elevational view, partly in section along the line 39—39 of FIG. 38;

FIG. 40 is a fragmentary sectional view taken along the line 40—40 of FIG. 37;

FIG. 41 depicts a sectional view taken along the line 41—41 of FIG. 39;

FIGS. 42A, 42B and 42C are top plan fragmentary views of the front end of FIG. 37 adjacent the electrical work coil to show the sickle sections progressively approaching the work coil;

FIG. 43 is a diagrammatic view of the electric circuit associated with the machine illustrated in FIG. 37 and showing the controls;

FIG. 44 illustrates another embodiment of the endless chain type for carrying the invention into practice and for armoring saw teeth shown in FIGS. 10 to 12;

FIG. 45 is a sectional view of fragmentary character taken along the line 45—45 of FIG. 44 to show a saw tooth and its support;

FIG. 46 shows a top plan view of FIG. 45 from the line 46—46.

FIG. 47 depicts another sectional view taken on the line 47—47 of FIG. 44;

FIG. 48 is a fragmentary side elevational view of the upper portion of the endless chain machine of FIG. 44, partly in section along the line 48—48, to illustrate saw teeth approaching the end of the cycle and also a finished armored saw tooth dropping into a discharge chute;

FIGS. 49 to 52 depict various armored articles of manufacture made by the improved induction method;

FIG. 53 is a diagrammatic view of a lay-out embodying the present invention for armoring a band saw;

FIG. 54 is a fragmentary perspective view of a part of an armored band saw;

FIG. 55 depicts another lay-out, diagrammatically illustrated, for armoring teeth of a hack saw or band saw;

FIG. 56 is a perspective view of an armored hack saw;

FIG. 57 shows still another lay-out, diagrammatically illustrated, for armoring the surface of a wire or rod;

FIG. 58 illustrates a plan view of an armored wire or rod saw adapted for utilization in a hack saw frame;

FIG. 59 is a perspective view of a piece of wire or rod showing the armor on the entire cylindrical surface;

FIG. 60 depicts a further diagrammatic view of a lay-out for armoring a flat anti-skid, wear resistant, cutting and/or abrasive surface;

FIG. 61 is a perspective view of an armored flat strip, bar or surface;

FIG. 62 is a side elevational view partly in section, of a rotary carousel-type or turn-table type of machine for armoring articles of manufacture, such as saw teeth, by the improved induction method embodying the present invention;

FIG. 63 illustrates a part of the rotary platform shown in the carousel or turn-table type of FIG. 62 with saw teeth in their mounted position;

FIG. 64 shows a control device for use in connection with the carousel or turn-table machine of FIG. 62;

FIG. 65 depicts diagrammatically an electric circuit for use with the carousel or turn-table machine of FIG. 62 and the control device of FIG. 64;

FIG. 66 shows a modified embodiment of the invention for manual operation for armoring sickle sections;

FIGS. 67 and 68 illustrate further modified embodiments for manual operation for armoring other articles of manufacture, such as saw teeth and chip breakers;

FIG. 69 is a further modified lay-out for armoring the edge of a strip, bar, etc., to make a cutting tool, etc.

FIG. 70 depicts another modified lay-out for armoring a feed screw for use in feeding plastic, etc., in an extrusion press or other machine;

FIG. 71 illustrates the position of the electrical work coil around the front edge of the feed screw as viewed from line 71—71 of FIG. 70;

FIG. 72 is a diagrammatic view of an electric circuit

used in the present invention with a sensing device for producing improved results;

FIG. 73 shows a lay-out for armoring a rotating or rotary cutting device, such as a disc cutter, especially adapted for cutting concrete, cementitious materials and the like;

FIG. 74 is a perspective view of an improved electrical work coil, especially adapted for use in armoring the disc cutter shown in FIG. 73;

FIG. 75 is a sectional view taken along the line 75—75 of FIG. 74;

FIG. 76 depicts a fragmentary view, partly in section, taken along the line 76—76 of the work coil of FIG. 74;

FIG. 77 illustrates an improved electric circuit for use in connection with the work coil of FIG. 74;

FIG. 78 shows a perspective view of another electrical work coil, especially adapted for use in armoring teeth of a hack saw or the like;

FIG. 79 is a sectional view taken along the line 79—79 of FIG. 78;

FIG. 80 illustrates a perspective view, partly in section, taken along the line 80—80 of FIG. 79; and

FIG. 81 depicts diagrammatically an electric circuit used in connection with the work coil of FIG. 79.

In accordance with the present invention, an improved method is provided for applying in situ a hard refractory surface containing diamond substitutes to metal articles, such as, for example, ferrous or steel tools in a novel manner. The hard refractory surface is thin and when applied by the present method, it almost conforms exactly to the shape of the article, such as a steel tool. It likewise produces a sufficiently smooth surface so that for many purposes no smoothing operation is necessary. Generally, no grinding is required to re-shape the tool. Moreover, the hard refractory surface material and base metal fuse and/or bond at the interface, thereby giving an excellent bond and obviating most of the danger of chipping and shearing while at the same time retaining the hard surface containing the diamond substitute. When hard refractory or diamond substitute particles are of the carbide type, for example, and the base metal is of the ferrous type, for example, the constituents are soluble in the matrix alloy and thus provide an excellent bond at the interface. An armored tool, for instance, having an applied hard refractory surface, after subsequent normal heat treatment for the tool as if unarmored, has a finished surface apparently unaffected by the heat treatment.

Generally speaking, the present invention contemplates providing a thin, flat, hard armor on a metal article, such as a ferrous tool usually made with a base of steel, malleable iron, alloyed iron, cast iron or the like. The metal article is first cleaned in any appropriate manner to produce a metallic surface to which the armor will adhere tenaciously. For example, the base metal may be cold rolled or hot rolled which is pickled in a bath of a pickling solution and is then aggregate blasted. When cast iron is used, it is pickled and is then aggregate blasted or tumbled or milled; or when forged steel is used, it is aggregate blasted or tumbled. After suitable cleaning, the article or a selected surface or surfaces thereof has a film of liquid adhesive applied thereto. The adhesive application may be by brushing, spraying, dipping, printing or in any other appropriate manner. Such an adhesive film is then coated with a thin layer or coating of metal powder ground or granulated through a wide range of mesh, such as 5, 10, 20, 30, 40 or 50 down to 100, 200, 300 or 325 mesh. Powders of this kind can be obtained on the market or can be milled as those skilled in the art know. Metal powder for my improved induction process must soften or become plastic over a wide range of temperatures as in the illustrative examples disclosed herein and must not melt quickly and run away from the surface, particularly those which are sloped, inclined, vertical, irregular, internal, external, etc. Any excess powder is removed from the article or the surface

being armored. An effective and satisfactory way to apply powdered metal particles is to pass the metal article through a curtain of particles falling from a magnetic feeder or vibrating mass.

After the removal of any excess, the remaining powdered metal particles are held or retained tightly by the adhesive. Such remaining metal powder substantially constitutes a thin film which practically represents substantially a single layer. The coated article is preferably dried in any appropriate manner well known to those skilled in the art. When the article is dried, it is then ready to be heated in order to produce the permanent armor on the surface under treatment.

It has been found that my improved induction method of heating, which concentrates intense heat on the surface or skin of a selected area and which may be used without a protective atmosphere, is the most satisfactory and desirable when carrying the invention into practice on an industrial scale for the manufacture of commercial products. During such induction heating, the dried adhesive is volatilized and is replaced or displaced by the matrix constituent of the powder constituting a coating alloy which forms a permanent fusion bond between the armor and the surface of the metal article.

The temporary adhesive or binder has a volatile Such an adhesive or binder can contain suitable ingredients or the like, which can be volatilized and dried readily. such an adhesive or binder can contain suitable ingredients like shellac and borax. As those skilled in the art know, borax is a non-volatile, non-metallic, inorganic adhesive material which has plastic holding properties at the fusion bonding temperature of the matrix.

As an illustration, an alloy sold under the trade name Stellite may constitute the metallic matrix alloy of the armor which is fusion bonded to the article. When a diamond substitute is included in the armor, a carbide or carbides of refractory metals can be used such as one sold under the trade name Haystellite. For special purposes, cutting diamonds or the like may be used as those skilled in the art appreciate. In view of the high cost of cutting diamonds, they will be used only under special conditions where the service requirements of cutting are such as to justify the additional expense.

When special heat treating of the article is necessary, it may be immediately quenched in an appropriate bath and subsequently tempered to desired toughness. For instance, when steel is used, especially one which is suitably alloyed, the quenching may be effected while the article is still above a critical temperature.

In cases where it is desired to remove the glaze of fused borax from the surface of the metal article, it may be washed, for instance, in hot soda or other solution or in plain hot water. Whenever it is desired, a rust inhibitor may be added to the solution or the water. After washing, the metal article may be subjected to wire brushing, tumbling or the like.

A detailed description of my armoring process or method is broadly and generally disclosed in my co-pending patent application Ser. No. 546,779, filed Nov. 14, 1955 (now U.S. Patent No. 3,023,490) and a detailed description of my armored product produced by my armoring process or method is disclosed in my co-pending application Ser. No. 548,915, filed Nov. 29, 1955 (now U.S. Patent No. 3,024,128). The disclosures in these co-pending patent applications are incorporated herein by reference. By so doing, the description given herein will be simplified.

In carrying the invention into practice, those persons skilled in the art will understand that any appropriate equipment may be used or any suitable arrangement or combination of pieces or units of machines or auxiliaries may likewise be employed. It has been found that for certain types of armoring special arrangements and combinations are desirable as satisfactory results have been produced. For most desirable operations and for best re-

sults, it is preferred to use the equipment, the arrangements and the combinations set forth and illustrated herein.

For the purpose of assisting those persons skilled in the art to carry the present invention into practice, a flow sheet has been illustrated in FIG. 1 of a combination of operations which can be conveniently used. It is to be understood, however, that the combination of operations and the like illustrated in FIG. 1 merely constitute one embodiment of the invention. As those persons skilled in the art know, various modifications of the operations and the like may be resorted to whenever it is deemed desirable under industrial conditions of manufacture or for the production of certain commercial articles, products, parts, tools and the like.

In the flow sheet illustrated in FIG. 1, the reference character "A" designates the first operation which usually has to be conducted, especially with articles, products, parts, tools and the like made of various metals and alloys which are delivered from the open market or obtained from storage, etc. For convenience, such an article, product, part, tool or the like will be termed a "work piece." In the ordinary course of events, the work piece is usually subjected to a cleaning operation. As is well known in the art, such a cleaning operation may vary according to the source and nature of the metal or alloy constituting the work piece. In the event that the work piece is constituted of an iron base or a ferrous alloy or a steel, then it is desirable to pickle the work piece in a suitable pickling solution known to and/or available in the art to remove scale, oxide and the like from the exterior surface. Thereafter, it is usually desirable to subject the pickled work piece to aggregate blasting to produce a good surface receptive for armoring. Before the aggregate blasting, it is preferred to wash the pickled work piece with water or with any other kind of suitable solution (e.g. alkaline or soda solution), to remove the remains of the pickling solution on the surface of the work piece and to neutralize any acid remaining from the pickling solution.

The second operation is designated by reference character "B" and involves the application of an appropriate film of suitable adhesive to the surface of the work piece. To facilitate the application of the film, the adhesive is preferably converted to a liquid or fluid condition. By so doing, the liquid or fluid adhesive may be applied in any convenient manner. For instance, any mode usually employed in the paint or printing industries may be utilized. Thus, the film of adhesive may be applied by brushing, spraying, dipping, printing or in any suitable way selected by a person skilled in the art.

After the application of the adhesive film on the work piece, the next operation designated by the reference character "C" in the flow sheet may be carried out. This operation involves the distribution of a powder on the adhesive film. Such a powder may comprise granulated or powdered metal and/or alloy and a flux. It is preferred to incorporate in the powder at least one refractory carbide, such as tungsten carbide, and at least one metallic matrix alloy. A refractory carbide powder which gave satisfactory results is one available on the market and sold under the trade name Haystellite and a satisfactory metallic matrix alloy is one also available on the market and sold under the trade name Stellite. It was found that a flux which produced satisfactory results was one containing borax alone or supplemented by boric acid, etc., and sold under the trade name of Oxweld Braze Flux. The amount of powder applied to the adhesive film depends upon the purpose of the work piece and the service conditions to which it will be subjected as those skilled in the art will readily understand. Similarly, the amount of refractory carbides to supplement the matrix alloy will be dependent upon the use to which the armored work piece is to be put. For mere hardness for wear resistance or for protection of a cutting edge of a tool, a smaller amount will be used than the case where the primary function of

the work piece is for its abrasive action or its cutting action. Naturally those persons skilled in the art may select the amount according to the use and service conditions as will be well understood by those skilled in the art. In some instances, a thin layer or approximately a single layer of powder may be used. In any case, excess powder which is not desired is removed in a suitable manner. The distribution of powder to the adhesive film on the surface of the work piece may be conveniently effected as by sprinkling through a screen and the like. A very convenient way giving satisfactory results was to pass the work piece through a curtain of particles of powder falling from a magnetic feeder or a vibrator or the like.

In the event that flux has not been incorporated in the powder as described hereinbefore, then operation "D" is used. The powdered work piece has its surface coated with flux, preferably as a powder. Coating of the surface may be done in any suitable way selected by a person skilled in the art. For instance, when a granulated or powdered flux is employed, sprinkling may be utilized or the work piece may be passed through a falling curtain of powder from a magnetic feeder or the like.

To facilitate the production of armored products, operation "E" may be preferably used in the flow sheet. The coated work piece is dried with any appropriate equipment. For example, the work pieces may be passed through an electrical heater or passed under infra red electrical lamps. In this manner, the coated work pieces may be dried thoroughly. When the operation of drying is conducted carefully, the powdered coating adheres tightly to the work pieces.

For the purpose of conveniently handling the work piece, it is arranged, placed or set on a refractory pallet as in operation "F." Such a refractory pallet can withstand the high temperature involved in induction heating. The pallet may be moved from position to position or can be carried from place to place by mechanical means, such as turn-table, a continuous conveyor chain and the like. It is preferred to place the work piece in some instances on a water-cooled copper fixture which will maintain a substantially constant temperature and which will also provide a shield to block the inductive field from the area not requiring heat. In this manner, the heat is restricted to the precise area which is to be armored.

In order to produce armor, the coated work piece must be subjected to inductive heat either partially or wholly in operation "G." Usually, a selected area of the work piece is inductively heated. By controlling the induction heat, the skin or thin surface of the selected area may be heated instantaneously and can be brought to a sweating temperature. Such heating occurs in a short period of time, usually a fraction of a minute or within a relatively few seconds. It has been found that the improved induction method of heating concentrates intense heat on the skin or surface and facilitates the control of heat to a sweating temperature where fusion of the armor occurs as well as bonding it tenaciously to the surface or skin of the work piece. When the work piece is subjected to induction heat, the formation of the armor and the bonding thereof occurs so quickly that it may not be necessary to use a protective atmosphere around the work piece. As a result of the induction heating, adhesive is dissipated and is replaced or displaced by the matrix alloy of the powder which forms a permanent fusion bond between the armor and the surface or skin of the work piece. Substantially the entire exterior of the work piece or the selected area is completely enveloped within a glaze of flux, such as a borax or borate glaze. This protects the hot armored work piece from detrimental influences in the surrounding atmosphere.

The hot armored work piece may be allowed to cool by itself. However, for practical operations, particularly on an industrial scale for the production of commercial articles and products, a cooling operation "H" is usually

employed. Various types of cooling equipment may be used, such as jet spraying liquid or air on the surface of the hot work piece. Instead of a spray, a quenching tank filled with a liquid may also be utilized. For practical operations, especially in the armoring of steel work pieces, a variety of quenching media is available. Usually, water or oil is preferred, but other media may be substituted, such as molten salt baths and the like. By using an appropriate bath of suitable quenching oil, the hot work piece may be properly heat treated and then subsequently tempered to the desired toughness. It is well known to those skilled in the art how steel and particularly alloy steel may be heat treated and the like.

As a general rule, it is ordinarily desired to remove the glaze or any loose material from the armored work piece. Removal of the glaze and loose material can take place in any convenient way. Usually, it is sufficient to wash the glazed work pieces in water or alkaline solution (e.g. hot soda solution). As those skilled in the art understand, removal operation "J" may also be effected in various other ways, such as tumbling, wire brushing, shot blasting and the like.

In those cases where the work piece has a cutting edge or requires the formation of a cutting edge, operation "K" can be conducted in an appropriate manner. In the event that the work piece initially had a cutting edge, it merely has to be restored to a cutting condition. When the work piece had no cutting edge or only a "blank" one, it has to be machined, ground and the like to a final cutting edge as those skilled in the art appreciate.

The production of an armored work piece is depicted in the final operation "L" of the flow sheet. Such an armored work piece may possess various advantages and beneficial properties. Thus, the final armored work piece 35 may be hard, wear-resistant, abrasive or abrasive-resistant, sharp with cutting ability and the like or may have a cutting edge protected against wear.

The operations and the like shown in the flow sheet of FIG. 1 have been illustrated diagrammatically and in detail in FIGS. 2 to 12. Thus, a work piece (e.g. a sickle section or blade) is depicted as being cleaned in a suitable bath held in a container. The application of a film of adhesive to the surface to be armored is effected by means of a spray as may be seen in FIG. 3. Powder may be sprinkled on the adhesive film on the surface of the work piece as shown in FIG. 4 by shaking it under a screen. Similarly, flux may be sprinkled on the adhesive film (see FIG. 5). For conducting the drying operation, a bank of infrared electric lamps may be used as diagrammatically illustrated in FIG. 6. The coated work piece (e.g. sickle section) may be seen in FIG. 7 where it is associated with a refractory pallet and where it is ready for fusion and bonding. In FIG. 8, an electrical work coil is depicted with the work piece in position to be inductively heated to effect instantaneous fusion of the armor and bonding to the surface of the work piece. Cooling the work piece may be effected by blowing or spraying air or a liquid against the hot surface (see FIG. 9). Removal of loose material, flux glaze and the like may be conveniently done by means of a pair of rotating wire brushes as shown in FIG. 10. As may be seen in FIG. 11, an armored saw tooth may have its cutting surface prepared by grinding. In FIG. 12, the ground armored saw tooth is depicted. It will be observed that the armor only covers a selected area of the saw tooth which protects the cutting edge in this illustration.

For the purpose of inductively heating a work piece, any appropriate or suitable electrical induction heating apparatus, equipment or machine which is well known in the art may be used. Electrical power may be obtained from any convenient source. Usually, for practical, commercial and industrial purposes alternating electric current is provided by high tension electric power lines coming from a public utility power plant. Generally speaking, 75

three phase alternating current is delivered by the electric power line as shown diagrammatically in FIG. 13. By means of a transformer "T," the voltage is changed to a desirable or preferable level. Thereafter, the high frequency electricity is rectified in a rectifier "R" of well known construction and operation. The rectified electric current goes to a well known oscillator and tank circuit "O" which supplies an electrical work coil "W" with electric current at an appropriate voltage and current. In the work coil, a work piece is inserted (see FIG. 8) to be heated inductively and to cause fusion of the armor and bonding it to the surface or skin of the work piece.

While the present invention may be carried into practice with any appropriate and suitable machines, electrical circuits, electrical devices and induction heaters as those skilled in the art understand, it is preferred to use those illustrated in the drawings (see FIGS. 14 to 81.) Thus, various figures in the accompanying drawings depict machines, electrical devices and electrical circuits which have been found satisfactory to carry my improved induction method into practice.

Referring more particularly to FIG. 14, a foundation plate or base 1002 supports all of the devices utilized in applying a coat of adhesive to a selected area of a metal article of manufacture (e.g. a sickle section or blade) which is to be armored. On the right-hand side of the foundation plate or base, a fixture block 1004 is anchored and secured by suitable means, such as screws, which extend through adjustment slots 1008. The fixture block is arranged to support and hold the article of manufacture in position. It will be observed that a sickle blade or section 1001 is illustrated in dotted lines at the right-hand end of the figure.

An adhesive pan 1005 is mounted on the foundation base to the left of the fixture block. To adjust the location of the pan with respect to the block, a locating strip 1003 and adjustment screws are used. In the pan, a felt pad 1006 is placed as may be clearly seen from FIG. 14. Liquid adhesive 1007 is filled in the pan and extends to near the working surface of the pad, say about one quarter of an inch or so. In this manner, the pad is kept saturated with liquid adhesive and the surface thereof is furnished with a supply. To transfer a small amount of this supply of liquid adhesive to the area to be coated on the article, appropriate transfer means, such as brushes 1011, are provided.

The detailed construction of the brushes may be clearly seen from FIG. 18. A brush fixture block 1028 holds brushes 1011 in a downward vertical position. This brush fixture block is held at the end of a mounting bar 1009. Any suitable means may be employed for holding the fixture block, such as a plurality of screws 1029A which fit into a plurality of threaded mounting screw holes 1029B. These screw holes are counter-bored to accommodate springs 1027. By providing these springs, tension may be put between mounting bar 1009 and the brush fixture block 1028 and adjustment of the bottom of the brushes may be effected with respect to the area on the article to be coated.

The mounting bar 1009 holds the brush assembly at one of its ends and is secured at its other end to a channel plate 1010 by a plurality of screws 1014. Identical radii plates 1015 are rotatably fastened at their upper ends 1016 to mounting bar 1009 and at their lower ends 1016 by means of self-centering screws 1017 and nuts 1017A. Center bushings may be provided at the upper and lower ends where the screws engage the radii plates 1015.

At the lower ends, plates are rotatably fastened to a base carriage assembly plate 1018. As may be clearly seen from FIG. 16, this construction provides a parallelogram hinge and slide. This parallelogram construction is hinged at its corners and is capable of imparting an arcuate motion to carry the brush assembly from the felt

stamping pad 1006 in pan 1005 to the surface of the area of the article to be coated with an adhesive.

The base carriage assembly plate 1018 is fixed to slide bars 1019 which are adapted to slide in grooved ways 1020. These ways are secured to the foundation base or plate 1002 in any suitable manner, such as a plurality of screws illustrated in FIG. 17. To adjust and limit the travel of the carriage assembly in its sliding forward motion in the grooved ways, an adjustable bumper 1021 is provided as may be seen in the right side of FIG. 16. On the left side, an adjustable limiting bumper is likewise provided. To cushion and limit the reverse sliding motion, a spring 1035A is mounted at the end of bumper 1035 (see also FIG. 19 for view of details). Such action keeps the felt pad 1006 from getting its surface too sloppy when brush 1011 lands on it and also eases any spatter.

At the end of the sliding forward motion, adjustable screw bumper 1022, which is attached to bar 1023 as shown in FIG. 14 actuates micro-switch 1024 which energizes relay 1025 (see FIG. 23). When relay 1025 is energized, it causes a reverse sliding motion. The energization of relay 1025 is continued until the end of the reverse motion. The normally closed micro-switch 1026 is opened by an adjustable bumper screw 1036 which is attached to bar 1023 and which causes relay 1025 to be de-energized. After de-energization, the forward motion circuit is ready to be energized and actuated by switch 1012 which is depressed by an article 1001 when placed on fixture 1004 (see FIG. 14). To locate the article in its proper place on the fixture, a plurality of pins 1013 is provided as clearly shown in FIGS. 14 and 15.

The foregoing construction imparts suitable sliding motion which enables brushes 1011 to be properly wet with liquid adhesive. After proper wetting, the brushes are raised up and out of pan 1005 and are swung in an arc by means of arcuate motion. This motion continues until the brushes are brought into contact with the article 1001. Upon the return motion, the brushes are subjected to a sliding action and are caused to wipe the area of the article to be covered with adhesive. Reference to FIG. 15 will reveal the brushes 1011 positioned in the upper location of article 1001 just prior to the occurrence of the wiping action. By effecting the sliding action, an even, bubble-free adhesive coating, layer, film or the like is applied.

For effecting the motion of the brushes from the pan to the article and return, pneumatic or hydraulic pressure may be used. Such pressure can be controlled through a double-acting solenoid valve 1030 (see FIG. 14). Thus, the forward motion is controlled by the pressure from the source. The reverse motion, however, necessitates a soft drop of the brushes on to the pad. For controlling the reverse motion, a direction valve 1031 is provided which reduces the reverse motion speed. Such controlled flow imparts movement to carriage plate 1010 through cylinder 1032. To open and close the electrical circuit to the power lines supplied by a utility or other source of electricity, an electrical switch 1033 is provided (see FIG. 14).

The operation of the adhesive applying machine will be readily understood by those skilled in the art. For convenience, however, the following description will be given.

An article of manufacture, such as a sickle section or blade 1001 is set firmly on the fixture block 1004 and against the locating pins 1013. In this position, the sickle section or blade is over the micro-switch 1012 lever arm so that the lever arm is depressed. This activates the forward motion of the carriage (see FIGS. 16 and 17). As the carriage moves forward, the base of the carriage 1018 slides in its grooved ways 1020 thereby causing brushes 1011 to slide on the adhesive pad 1006. The sliding motion of the carriage base 1018 is stopped by an adjustable limiting bumper 1021. At this time, the carriage is arcuated up and out of pan 1005 in such a manner that the brushes 1011 swing through that arc. In this movement,

the working surfaces of the pad 1006 remain substantially parallel to the section 1001 hold on fixture block 1004.

At the end of the path of the arc, the brushes 1011 are placed on the sickle section 1001 and are immediately actuated in the opposite direction by bumper 1022 depressing switch 1024. At the start of this reverse traverse, the weight of the carriage permits the base 1018 to travel in its grooved ways 1020 to the opposite adjustable bumper 1021. This causes the brushes 1011 to slide on the selected area of the sickle section 1001 to cause the application of a uniform, a bubble-free coating or layer of adhesive. Upon contact with the reverse traverse bumper, the brushes 1011 are arcuated up and off the sickle section. At the end of reverse arcuate path, the brushes are dropped onto adhesive pad 1006 while simultaneously bumper 1036 actuates switch 1026 to make ready for another cycle.

As soon as brushes 1011 leave on the reverse traverse, the sickle section 1001 is removed and immediately passed at an angle through a curtain of particulate armoring material falling from a magnetic feeder (e.g. a Syntron Feeder) and then directly passed through a curtain of particulate flux falling from the magnetic feeder. The coated sickle section is now ready for the fusing operation to be performed by an induction heating machine to be described hereinafter.

The construction of the induction machine and associated auxiliaries and equipment will be obvious to those skilled in the art from FIGS. 24 to 35. For convenience, however, the following description will be given.

A base 8, such as a steel plate or the like, is used for mounting a plurality of legs 4, 5, 6 and 7. Fixed to the top of the legs is a pair of slideways 24 for carrying articles of manufacture, such as sickle sections or blades, or other parts which are to be armored in whole or in part. Carriage slide bars 27 are mounted in holes bored in the legs.

The carriage may be clearly seen in detail in FIGS. 25, 26 and 30. Base beams 28 are provided with bushed holes 65 to permit them to slide on slide bars 27. Piston rod 30 operating in cylinder 37 is attached to the carriage by means of bracket 31 (see FIG. 24). Bushed posts 29 are attached to beams 28 to carry risers 25 and plate 48 (see FIG. 31). The risers are designed to support a plurality of posts 44, 45, 46 and 47 which carry the indexing bars 23. Strips are mounted on beams 28 to provide centralized ways in which slide bar 35 can slide. Attached to slide bar 35 are camming wedges 42 which move between risers 25 (see FIG. 31). This enables them to cam the posts and keep the indexing bars parallel as they move in and out. Springs 49 hold the risers to ride against the camming surfaces of the wedges. Cylinder 34 is attached to a plate 48 with its piston rod 39 connected to a wedge bracket 40. This construction enables the wedges to cam risers upon pressure being applied in the proper direction to cylinder 34.

A plurality of switch-tripping screws 13, 38, 50 and 55 and a cam 58 are carried by strip 22 which is attached to carriage beams 28. Bar 16 is slotted for electric switches' moment adjustment and attached to legs 5 and 6 in a position parallel to the travel of the carriage as may be clearly seen in FIG. 24.

An adjustable screw 38 is positioned to cam micro-switch 36 on leg 5. A cam 54 on post 44 is positioned to cam switch 55 when moved by camming action of wedges 42. An adjustable screw 13 is positioned on and adjusted to cam directional switch 14 which acts only during the forward phase or movement of the carriage. An adjustable screw 50 is positioned to cam "heat-on" directional switch 51 which acts only in the reverse phase or movement of the carriage. Holding cam 58 is mounted so as to cam normally closed holding switch 12 which is positioned in its slot so as to be held open until switch 51 has been actuated. An adjusting screw 56 is positioned and adjusted to actuate switch 33 to remove wedges 42. To adjust

the limit of the forward phase or movement of the carriage, an adjustable limiting screw 53 is provided which is mounted in girt 53G.

Fixture block 21 is mounted on a dielectric beam 9 which is attached to the table top 3 and supported by post 41. The working surface of the fixture block is in the same plane as the working surface of slideways 24 (see FIG. 27). Dielectric beam 9 electrically insulates the fixture block 21 from the rest of the mechanism. Fixture block 21 is made of copper and shaped in a manner to keep the desired area of part 19 from being heated by shielding the desired area from the action of the inductance of work coil 32. To keep the fixture block cool, it is pre-cavitated to permit cooling water to flow through it. Likewise, electrical work coil 32 is shaped to the proper geometry and coupled in a suitable manner to provide a desired heat pattern on the article or part 19.

Indexing bars 23 are equipped with lugs 26 and are caused to walk along slideways 24 in such a way that the foremost part or article is pushed on the slideways by the lugs onto fixture block 21. This is designed in such a manner that a magnet 20 which is inserted in its surface, holds the part or article 19 firmly against the surface of the fixture so that any foreign material is pushed off by the part or article and cannot build up to give any trouble. Magnet 20 also causes a firming and braking action to hold the part or article against lugs 26 to accurately fixture the same on the fixture block. To further assure the accurate fixturing, clamp 18 is adjusted so that it engages the part or article before it is entirely pushed into position on the fixture block 21. The clamp is operated by cylinder 17. This braking action assures positive fixturing in work coil 32.

Hangers 66 hold coil 32 in proper position and facilitate adjustment to provide the desired heat pattern for effective fusing or bonding the armor to the base. Adjustable coil hangers 66 are attached to dielectric mounting board 57. For convenience, other things were assembled on the mounting board.

After the instantaneous heating of the article or part by the induction heater, the armored article is ejected from the electrical work coil 32 and the fixture block 21 by fingers 52 which are mounted on and extending beyond bars 23 onto fork 59 during the forward phase or movement of the carriage (see FIG. 30). As the carriage moves in its forward phase, adjustable bumper screw 61 travels forward with the carriage until it bumps push rod 62 thereby causing fork 59 to move in an arc around its fulcrum 60. Universal joints 63 and 64 make connections between push rod 62 and pick-up fork assembly 59.

As counter balance 43 and pick-up fork assembly 59 are pushed past their center balance, they pick up speed and cause push rod 62 to be pulled forward and to leave bumper screw 61. A collar is positioned on push rod 62 so that the forward motion of the pick-up fork will be suddenly stopped thereby jarring the article or part from the pick-up fork into a "tote pan" or onto an appropriate chute to be slid into a suitable quenching medium. Then, upon the reverse traverse of the carriage, the collar carries the pick-up fork back into a loading position (see FIG. 30).

The electrical circuit is shown in FIG. 35. The numbers of the switches in FIG. 24 indicated their positions. Electric switches 14, 33, 36 and 55 and the series combination of parts 10 and 12 and induction generator relay 95 operate cylinders 17, 34 and 37 through solenoid valves. Relay 95 is an extra installed in some induction generators for similar purposes.

Switch 10 is mounted in a convenient place on switch-mounting bar 16 along with push-button switch 11. It is to be noted that switch 10 is a single pole double throw type which is placed in a position to close the circuit through normally closed switch 12 and normally closed relay 95, thereby actuating cylinder 37, forward traverse solenoid valve and cylinder 17 to open clamp 18 and sole-

noid valve to start the automatic cycling of the carriage (see FIG. 30).

Forward traverse cam 58 has the function to open and hold open normally closed switch 12. Switch 14 is placed in position to enable it to actuate cylinder 17 to close clamp 18 and solenoid valve before the forward most traverse of the carriage so as to accomplish the accurate fixturing (see FIG. 30).

Switch 36 is actuated by adjustable bumper screw 38 which activates cylinder 34 to insert wedges 42 and solenoid valve thereby moving post 44 away from post 29 and causing cam 54 to cam switch 55 which actuates cylinder 37 to reverse traverse solenoid valve. It is to be noted that it is necessary that switch 14 not be closed as its camming screw 13 returns over it so that its lever arm is adapted to take care of this function.

As the reverse traverse of carriage continues, adjustable screw 50 cams directional switch 51 to close the timer circuit in the high frequency generator. This removes the grid bias thus turning on the heat for the "heat-on" cycle and also energizing relay 95 thereby opening the circuit for a forward traverse. When cam 58 lets switch 12 close, the carriage is held in the rearmost position until the grid bias is applied by the timer circuit when the heat is on and the time cycle is satisfied thereby relaxing relay 95 to cause recycling.

At the rearmost traverse, adjustable bumper screw 56 actuates switch 33 to activate cylinder 34 and to remove the wedge 42 and the solenoid valve. Switch 10 is adapted to function as a single pole double throw switch so that the other position will close circuit-making cycle possible through push-button switch 11 for servicing and adjusting.

From the foregoing description of the induction heater and associated auxiliaries and equipment, the operation will be obvious to those skilled in the art. Induction heating systems and high frequency generators are well known to the art and are disclosed in many prior patents and publications. Detailed description of such systems and generators is unnecessary and those persons skilled in the art are referred to prior patents and publications. For convenience, however, the following description will be given of the present improved method utilizing induction heating.

At the outset, the usual procedure for putting conventional high frequency source of alternating electric current into operational readiness is effected. The article of manufacture or part such as a sickle section or blade disclosed and illustrated herein, which has been coated in a manner described heretofore, is loaded between carriage indexing bars 23 properly oriented in front of lugs 26 on slideways 24. After initially loading the machine illustrated in FIG. 24, the starting switch 10 is now actuated to the automatic position. This activates the main indexing carriage in the forward phase. The articles or parts 19 are carried along the slide ways 24 into the next forward position with the foremost one entering the instantaneous fusing or bonding area in the work coil 32 on the fixture block 21. This block has a permanent magnet 20 inserted in its central surface and their fixturing surfaces are in the same plane and also in the same plane as the slideways 24.

As the article or part is sliding onto block 21, magnet 20 has a braking and firming action. To help this action just about at the end of the forward traverse, clamp directional switch 14 activates clamp 18 to assist this braking and firming action to insure accurate fixturing of the article or the part. Screw 13 activates the directional switch 14, which in turn, activates clamp cylinder 17.

The forward traverse adjusting screw 53 limits the motion and simultaneously therewith micro-switch 36 is bumped by adjustable screw 38 which senses wedge cylinder 34 and which slides wedges 42 in pushing indexing bars 23 apart so as to clear the articles or parts upon the reverse traverse via wedge cam risers 25. Cam 54 on the side of post 44 bumps switch 55 thereby cam-

ming it to sense the indexing cylinder 37 for the reverse traverse. During the reverse traverse, directional switch 14 is not activated. The adjustable screw 50 cams switch 51 sensing "heat-on" relays in the high frequency induction generating system. An adjustable bumper 61 at the rear end of the indexing carriage limits the reverse traverse and simultaneously adjustable screw 56 activates switch 33 sensing the cylinder 34 to remove wedges 42 and to allow indexing bars 23 to close for recycling. This recycling takes place when the extremely short period of time for fusion is satisfied through the generator sensing system which closes the generator relay which in turn senses cylinder 17 to open clamp 18 and cylinder 37 to cause forward traverse.

The starting switch 10 is in series with a normally closed relay in the induction generator and normally closed holding switch 12. When heat is on to cause fusion of the armor coating to the article or part, the generator relay is held open so recycling cannot occur until heat cycle is off, thus closing relay causing recycling. Heat being off during a portion of the reverse traverse, the carriage would immediately attempt a forward traverse at the forward most traverse, if it were not for holding switch 12. This holding switch is held open by holding cam 58 until "heat-on" switch 51 is activated.

The article or part, which has had its armor fused thereto in a selected area, is ejected from the work coil 32 by ejection fingers 52 onto the pick-up fork 59. This fork swings on fulcrum 60 which is pushed at the right moment by adjusting screw 61 on the carriage which bumps push rod 62 to which universal joints 63 and 64 are attached. Such action smoothly activates the pick-up fork 59 which carries the fused or armored article or part out of the work coil and deposits it into the chute for delivery to "tote pan" or into quenching medium according to the desire of the operator. Pick-up fork 59 is brought back by a collar or push rod 62 which is positioned so that the carriage pulls it on its return traverse. Counter balance 43 holds the proper position in the said motion during any "lost motion."

Electric switches 12, 14 and 51 may be adjusted to operate at the right moment by moving them along in their mounting bar slots. The adjustable coil hangers 66 are used to hold the work coil 32 in position and also to adjust the work coil so as to provide the proper heat pattern for effective fusion or bonding of the armor to the article or tool, etc. Starting switch 10 placed in another position makes push-button switch 11 operable for manual control for servicing and testing.

It will be evident to those persons skilled in the art that improved machine associated with the induction heater is an adaptation of automatic feeding to a high frequency source of electrical energy. The use of this machine and associated induction heater in connection with my improved method makes possible the processing of articles or parts to be heated in a specific and selected area or areas which a concentration of intense heat which is capable of fusing or bonding practically instantaneously the armor powder coated adhesively onto said area or areas and which effects an instantaneous fusion or bonding of the armor to the underlying surface of the article or part to be armored.

For the purpose of giving those skilled in the art a better understanding of the invention, the following illustrative examples are given to illustrate the organic adhesive which can be used to coat a selected area or areas of an article of manufacture or part to be armored and also to illustrate the powder mixture which can be used to armor the article or part.

tion constituting the organic adhesive is prepared as follows:

|                       | Percent by weight |
|-----------------------|-------------------|
| Orange shellac        | 3.75              |
| 80% denatured alcohol | 96.25             |

The shellac and alcohol are mixed to form a solution of the foregoing composition which is like those used in the paint art having a paint consistency and which is applied by dipping. As a general rule, it is preferred to add sufficient liquid, such as alcohol, to the liquid binder to make it thin so as to function like a liquid or fluid.

A powder mixture having the following compositions and constituting the armor for the article or part is formed as follows:

|                                  | Percent by weight |
|----------------------------------|-------------------|
| Flux                             | 11.4              |
| Stellite (matrix)                | 32.6              |
| Haystellite (diamond substitute) | 55.9              |

The powder contains particles having a range of sizes from about 100 mesh (about 0.0050" or 0.0059") to about 200 mesh (about 0.0025" or 0.0029"). The metallic components of the powder mixture constitute a non-eutectic type of alloy forming the matrix and having a substantial plastic or softening temperature range between the liquidus and solidus points below the melting point of the metal article and within a wide temperature range, such as somewhere within a range of about 1,500° F. to about 2,500° F., say, for instance, about 1,600°-1,800° F. to about 2,200° F.-2,400° F. The sickle section, for instance, with its surface coating of shellac-alcohol solution is passed through a fine curtain of the powdered material so as to coat the top and sides of the cutting portion of the sickle section or blade with the powdered material. The adhesively coated sickle or blade retains only a thin, uniform layer of the powdered mixture; the outer side of said layer being dry allows the excess powdered material to fall off or to be shaken or jarred off. This effects a removal of the excess of powdered or granulated coating mixture or alloy so that substantially a single layer is retained by the organic binder or adhesive film on the surface of said tooth or metal article. When the organic binder or adhesive is made of shellac solution, the viscosity of this solution must be taken into consideration with respect to the thinness of the film of adhesive and the layer of metal powder constituting the armor.

The sickle blade with the powdered layer held in place by the shellac solution, which dries rapidly, is heated after drying in the induction machine to the sweating temperature, i.e., one which is above the melting or softening point or range of the matrix material whereupon there is a fusion or bonding at the interface of the surface layer and the ferrous base of the sickle blade or tool by melting or fusing or bonding. In this heating operation, the surface of the sickle blade or tool is heated to a temperature within the aforesaid plastic range at which said coating alloy will displace said non-metallic adhesive material (for example, borax and/or boric acid and/or mixtures thereof) and will fusion bond with the surface of said sickle blade or other tool or metal article. The shellac binder is subject to pyrolysis during heating and the flux, which is preferably borax in part, takes over the function as binder and holds the carbide grains in place and protects them from oxygen. Borax functions as a non-volatile, non-metallic inorganic binder or adhesive material with plastic holding properties at the fusion bonding temperature. A smooth thin hard layer of armor is formed on the surfaces treated so as to accurately reproduce its contour. The armor is tightly bonded to the remainder of the sickle blade and requires no grinding operation. A borate glaze envelops the armor and protects it from detrimental effects of the surrounding atmosphere. The sickle blade can be heat treated just as though

#### EXAMPLE I

An alcohol-shellac mixture of the following composi-

the surfacing had not been applied and will substantially retain its hardness.

As indicated hereinabove, the composition of the final surface layer should be determined by the conditions of use to which the article will be subjected. For example, where the shock which the sickle blade or tool is to meet is not too great, silicon carbide or boron carbide are preferably included. Such a product is particularly useful for abrading and/or cutting surfaces.

A sickle blade or section manufactured in accordance with the foregoing example has a hard thin surface of armor which is self-sharpening during use; has a relatively smooth, hard surface when initially applied requiring no grinding on the coated surfaces prior to use; is produced by a method more quickly, easily and inexpensively applied than by methods heretofore known; wears from many times as long as sickle blades which have not been hard surfaced; may be heat treated without rupturing the bond between the ferrous article or tool and the hard surfacing; retains during normal heat treating of the ferrous article or tool the desirable quality of hardness of the hard surfacing; is relatively free from tendency to chip or shear off the hard surfacing during use; and is created by a process resulting in a substantial saving of materials over methods previously known. Of course, the proper cutting angle should be maintained on the cutting tool, especially when it is worn and/or when it is restored. This is accomplished by grinding on the face in a manner well known to those persons skilled in the art.

#### EXAMPLE II

The proportions set forth in the foregoing Example I can be varied, but are preferably of the following order:

Wet portions of the organic adhesive or binder:

|                       | Percent by weight |
|-----------------------|-------------------|
| Orange shellac        | 2-4               |
| 80% denatured alcohol | 96-98             |

Dry portion containing the armoring constituents:

|                                  | Percent by weight |
|----------------------------------|-------------------|
| Powdered sugar (optional)        | 0.05-0.5          |
| Borax (flux)                     | 5 or 10-10 or 15  |
| Stellite (matrix)                | 30-40             |
| Haystellite (diamond substitute) | 50-65             |

The dry portion is composed of powder having a size range varying from about 20 mesh (about 0.30" or 0.033") to about 300 mesh (about 0.001" or 0.0017"). The matrix metal powder may likewise vary from about 30 mesh (20 microns) to about 325 mesh (44 microns). Of course, the flux is screened to obtain the same size range.

In lieu of borax together with calcium chloride and zinc chloride, or either calcium chloride or zinc chloride together with borax, a suitable commercial borax mixture may be used. For instance, a suitable one is sold under the trade name of Ozweld Brazo Flux. Analysis shows this commercial flux consists mainly of a borax mixture and may contain boric acid. The constituents of the flux give fluidity to the heated materials, tend to lower the melting point of the high melting oxides, and provide protection against unwanted oxidation. As those skilled in the art know, a flux functions in a number of ways including covering or enveloping the surface or surfaces to protect them from oxidation by the atmosphere while heating, dissolving any oxides formed on the metallic surface or surfaces, and lowering the surface tension of the molten, softened or plasticized matrix to allow it to flow or spread sufficiently to coat all adjacent parts, surfaces and/or particles and to form a fusion bond at the interface of the metal base and the armor or coating. The flux forms a protective glaze over the armor like a glass envelope.

The temperature and humidity at the time of application will affect the proportion of alcohol in the shellac solution. Too little alcohol will result in balling up of the

10

5

15

20

30

35

40

55

60

65

75

material on the surface of the tool to be coated and will result in an uneven application of the hard surfacing material. As well understood by those skilled in the art, the alcohol acts as a liquid vehicle.

Other carbohydrates, such as molasses and syrup, may be substituted for the powdered sugar, although sugar is preferred. Glue may be substituted for the shellac but does not seem to work quite as well. The temporary binder must be of a composition which does not decompose into volatile constituents too quickly. Molasses, syrup, or the like may also act as an adhesive with or without the shellac solution.

#### EXAMPLE III

Wet portions of organic adhesive:

Shellac, alcohol or shellac solvent.—Suitable proportions to form liquid or fluid adhesive to be applied by spraying, dipping, brushing or other ways known to the painting art.

Dry portions constituting the armor:

Diamond substitutes — Coarse granules (about 10,

20 or 30 mesh).

Diamond substitutes — Finer granules (about 200, 300 or 325 mesh).

Stellite — Matrix alloy.

Flux — Borax mixture containing boric acid.

#### The first operation

Article is coated with a film of shellac solution by any desired method known to the art of painting or the like, such as shown by the machine described herein for stamping a coat of organic adhesive on the area to be armored.

#### The second operation

Distribute coarse granules of a diamond substitute, such as refractory carbides, of a size that the thinness requires over the adhesive covered surface or surfaces in any desired pattern in order to get a substantially even distribution.

#### The third operation

Distribute a fairly coarse size of matrix granules over the coarse granules of the diamond substitute. This will cause a lesser amount of matrix to fall between the coarse diamond substitute granules so that after fluxing and bonding the coarse granules will protrude slightly.

#### Alternate to third operation

A mixture of 100 mesh and finer or any grain size required by the finished article of matrix alloy and diamond substitute which would fill up the spaces between the coarse granules of the diamond substitute and cause less protrusion of the diamond substitute.

#### The fourth operation

Overcoat the entire coating with a flux like borax which will function as a binder or adhesive until the matrix softens or fuses and becomes plastic.

A very thin coating of shellac solution should be applied before each operation if there is any evidence of insufficient wetting by the shellac solution previously applied.

#### The fifth operation

The coated article or part is subjected to intense heat by the induction machine which is concentrated in the selected area or areas to cause a fusion to the sweating point and of bonding the armor to the surface of the article, tool or part to be armored.

Another or equivalent machine for armoring sickle sections or blades is illustrated generally in a simplified form and on an enlarged scale with parts omitted for clarity to show how the sickle sections are advanced through the machine to the final armoring stage. An armored sickle section after being finished in the final armor-

stage is shown sliding down a discharge chute. As FIGS. 37 to 42C are generally similar to FIGS. 24 to 31, a detailed description will not be repeated. Those persons skilled in the art are referred to the description in connection with FIGS. 24 to 31 and the said description is incorporated herein by reference. Thus, in FIG. 37 a perspective view may be seen of a simplified machine generally illustrated in FIGS. 24 to 26 for armoring sickle sections, such as the one shown in FIGS. 21 and 22. Sickle blades are depicted as advancing through the various stages and then shown progressively approaching the electrical work coil and finally being positioned in the electrical work coil for armoring. FIGS. 38 and 39 illustrate sickle sections in three stages and FIGS. 42A, 42B and 42C show details of the three stages and the means for gripping and moving a sickle section from the first stage to the second stage and to the final stage where a sickle section is armored within the electrical work coil. FIG. 40 is a fragmentary sectional view of a part of the machine illustrated in FIG. 37 and FIG. 41 is a sectional view of a sickle section shown in the second stage in FIG. 37.

The operations involved in the machine for armoring sickle sections have been described fully in connection with FIGS. 24 to 31. However, some of these operations in connection with the electrical circuit and controls are illustrated in FIG. 43. Those skilled in the art will readily understand the electrical circuit and controls when taken in conjunction with the description of the operations set forth in relation to FIGS. 24 to 31. Thus, to start the operations, a switch is closed which is shown at the top of the electric circuit illustrated in FIG. 43. Switch "A" and the related parts of the circuit are depicted at the start of the operations and during the forward movement or travel of the carriage. Another switch illustrated adjacent to the "Power Line" is closed by the carriage at the end of the forward movement or travel. The closing of this switch energizes a solenoid which opens the index bars and actuates switch "A" and related parts for the return of the carriage. During the return travel or movement of the carriage a switch associated with the "Timer" is closed. After the return of the carriage, the operations are repeated again.

An endless chain type of machine is shown in FIGS. 44 to 48 which has been designed and illustrated especially for the armoring of saw teeth. A supply of such saw teeth 400S is depicted in the lower left-hand side of FIG. 44 on the supply tray 400T. An operator takes one of the saw teeth and places it in position on one of the links 400L of the endless chain designated generally by reference character 400C. This endless chain may be driven in any suitable manner, such as by the use of an electric motor 400M and associated driving means 400D as those persons skilled in the art will understand.

Throughout an intermediate region above the upper part of the endless chain, an electrical work coil 400K is mounted. During the passage of a saw tooth through and within the electrical work coil, it is inductively heated to a sweating temperature where the armor fuses and where the armor is bonded to the surface or skin of the steel base constituting the body of the saw tooth. After the formation of the armor and after the finishing of the armored steel saw tooth, it is removed from the link of the endless chain and is discharged into a chute 400H. This chute conveys the hot armored saw tooth into a collecting container 400N. Such a container is preferably filled with a quenching medium, such as water, oil or the like as well known in the art.

As may be seen from FIGS. 45 to 47, each saw tooth as it is carried in its link rides along on a refractory or insulating block 400B which is preferably made of a refractory ceramic dielectric material. It will be observed that the shape of the top of the refractory block conforms to the shape of the underside of the saw tooth. It is prefer-

red to incorporate or embed a part, say approximately one half, of the work coil in the refractory block as may be seen in FIG. 47. With this arrangement, the electrical flux passes directly through the tip of the saw tooth. In this manner the induction can be concentrated on a selected area of the skin or surface of the tip of the saw tooth which is to be armored. After being subjected to fusion and bonding, the hot armored saw tooth is cooled or chilled by the air. Such cooling or chilling insures instantaneous solidification of the armor and instantaneous bonding to the surface of the steel base. Thereafter, the armored saw tooth can be discharged into the chute (see FIG. 48) and conveyed to a container. This container, if desired, can be filled with a quenching bath (see FIG. 44). Subsequently, each armor saw tooth can be subjected to any other appropriate operations, such as heat treatment, sharpening and the like as those persons skilled in the art will appreciate.

Other articles, such as component steel parts and tools, are illustrated in FIGS. 49 to 52. The articles in FIGS. 49 to 51 are component parts and are adaptable for armoring in an endless chain type of machine or other suitable equipment. FIGS. 49 and 50 illustrate armored chip breakers whereas FIG. 51 depicts an armored chain saw tooth. In FIG. 52 a masonry drill is illustrated which is very useful in cutting or drilling holes in walls and other structural parts made of concrete, cement, stone, marble, cementitious material containing fiber glass and the like, etc. Of course, such drills can be armored manually or in a suitable machine for mass production.

A continuous armoring machine of another type is illustrated in FIG. 53. The embodiment of the invention is particularly adapted for the armoring or articles of manufacture like band saws. In this embodiment a coil 500C of unarmored band saw material is mounted at a raw material station in an appropriate manner. From the coil, a strip 500S of band saw material is withdrawn by means of a pair of driving rolls 500R. As the strip is moved, it passes underneath an adhesive station involving the use of a jet or spray 500J which applies a film, layer or coating of adhesive to the edge and top sides of the band saw. After the application of the adhesive, the strip is showered with falling particles of powder at a powdering station 500P. Such a powder has an appropriate composition and usually comprises metallic matrix alloy, diamond substitute and flux. From the powdering station, the strip is drawn along by a second pair of driving rolls 500R and is then bent through an arc of 180° to start a return travel or movement. To facilitate the return, a third pair of driving rolls 500R are mounted in alignment with the second pair.

During the travel of the strip from the powdering station to an induction heating station 500H, the adhesive has had an opportunity to dry and the powder is firmly adhered to the selected area of the band saw which is to be armored. In the event that it is deemed desirable, a drying station can be interposed between the powdering station and the induction heating station. Such a drying station may be equipped with appropriate auxiliaries, such as electrical heaters, infra red electrical lamps and the like, as well known to those skilled in the art.

When the dried strip passes through an electrical work coil 500W connected to a suitable induction machine (not shown) available in the art, the upper edge and adjacent sides are heated inductively to a relatively high temperature. This heating is controlled to a sweating temperature and is practically instantaneous. As a result, the armor is subjected to fusion and the armor is bonded to the skin or surface of the steel constituting the band saw. Over the armor is an envelope of a glaze of flux. Such a glaze protects the armored skin or surface from any detrimental effect of the surrounding atmosphere.

Following the armoring operation, the strip of armored band saw now travels into a heat treating station 500T. In this station, any thermal operation can be conducted

as will be understood by those skilled in the art. For instance, the hot armored strip may be cooled, chilled or quenched in a suitable medium. Thereafter, it may be subjected to any appropriate heat treatment to convert the steel into a desirable condition.

The heat treated band saw is withdrawn from the heat treatment station by a fourth pair of driving rolls 500R which are preferably mounted in alignment with the first pair. The withdrawn strip of armored band saw is wound on a second coil 500K which is mounted in a conventional manner and which may be driven when deemed desirable. Such a coil may then be handled in any desirable way. For instance, it can be cut into suitable lengths for making into bands for use in machines employed for cutting.

In FIG. 54 a finished piece of armored band saw is illustrated. It will be seen that the edge and adjacent sides are armored. It has been discovered that a more effective cutting tool is provided when slots are provided along the edge. An appropriate type of slot is shown in FIG. 54 as an oval one. By the use of slots or gaps 500G arranged at spaced intervals, the armoring is facilitated and the operating of a band saw is made more effective. Among other advantages, it may be noted that slots or gaps facilitate in removing and disposing of the material cut from the article, sheet, plate, etc., which is undergoing cutting by the armored band saw.

In the continuous armoring of a strip of hack saw blade, an arrangement shown in FIG. 55 will be found to be satisfactory. As may be observed in FIG. 55, a strip of hack saw blade 600S extends through a machine with a plurality of spaced stations which are adapted to perform special operations. The strip is supported by a plurality of driving rolls 600R. Whenever it is desired, these rolls may be driven. To keep the strip in proper alignment, a plurality of guide rolls 600G are mounted on each side of the strip and in engagement therewith. For controlling the speed of travel or movement of the strip through all of the stations and operations, main driving rolls 600M are in frictional engagement with the sides of the strip at the terminal end of the machine. These rolls are conveniently mounted and driven in the last station which may be designated as the driving station.

Adhesive may be applied to the teeth of the hack saw in any convenient manner. Thus, an absorbent porous roll 600A is supplied by liquid or fluid adhesive by a transfer roll 600T which in turn is in contact with a supply roll 600SR. This supply roll dips into the liquid or fluid adhesive contained in the supply bath 600B which is held in any appropriate container or tank. As the porous roll impresses adhesive onto the sharp corners of the teeth as well as the adjacent sides, more adhesive is supplied via the transfer and supply rolls. In this manner, a fresh supply of adhesive is available for application to the teeth of the hack saw.

As the strip of hack saw blade is moved along, it passes under a curtain of falling powder coming from a suitable vibrator or magnetic feeder 600F. Afterwards the adhesive is dried in an appropriate dryer 600D which may comprise electric heaters, a battery of infra red electric lamps and the like. The hack saw blade with the dried adhesive is ready to be inductively heated in an induction heater 600I. The electrical work coil is shown as positioned around and over the top of a portion or length of the hack saw blade. By controlling the induction heating, the instantaneous heat developed in the teeth of the hack saw blade can be controlled to a sweating temperature where the armor is fused together and is bonded to a selected area of the skin or surface of the teeth. Usually, the selected area is associated with the sharp corners of the teeth and adjacent side portions. The hot armored blade is passed through a cooling station 600C where water or a coolant may be introduced through one tube or pipe and withdrawn through another. Thereafter the cooled, chilled or quenched hack saw blade can be moved through

a heat treating station 600H where the blade can be subjected to any suitable thermal treatment. The finished armored hack saw blade is removed from the machine by the main driving rolls 600M.

After removal from the machine, the strip of armored hack saw blade can be cut into any suitable lengths. For instance, it can be cut into a length which will fit in the manual hack saw frame. Such a blade is provided with a pair of conventional holes as shown in an armored hack saw blade in FIG. 56.

For the armoring of cylindrical articles, such as wire, rods and the like, a machine (see FIG. 57) was designed which has been found to be convenient to operate and which has produced satisfactory results. A cylindrical article like a wire or a rod may be suspended from an upper bracket 700B on a mounting 700M. The lower end of the wire or rod may be held under tension by a weight 700W. To hold the wire or rod at a uniform distance from the mounting, a lower bracket 700L extends from the bottom of the mounting and encircles the lower end of the wire or rod. In order to move the wire or rod up and/or down, the mounting is fastened to a chain. As those skilled in the art will understand, the chain may be moved by gears or the like and an operatively associated electric motor. By controlling the speed of the motor, the speed of ascent or descent of the wire or rod may be controlled.

Before suspending the wire or rod from the upper bracket of the mounting, it is coated with an adhesive and then powdered with a powder. As an alternative, the adhesive containing the powder can be applied in one operation. In accordance with the usual procedure, the adhesive is preferably dried before subjecting the coated wire or rod to induction heat. This heat is applied by the use of an electrical work coil 700K which closely encircles the coated wire or rod. By moving the wire or rod at a controlled speed and by controlling the induction heat, the skin or surface of the steel wire or rod can be brought to a controlled sweating temperature where the armor is fused and the armor is tenaciously bonded to the steel base.

After armoring, the hot armored wire or rod can be cooled and then cut into convenient lengths, such as a length suitable for a hack saw frame and the like. A metal eyelet 700E can be joined to each end of the wire or rod by welding, soldering or the like as may be seen in FIG. 58. In case of need or desire, the finished armored wire or rod can be subjected to suitable heat treatment. A piece of the armored wire or rod is illustrated in FIG. 59 which shows that the cylindrical surface is armored throughout its surface. As a result, the armored wire or rod shown in FIG. 58 can be mounted in a hack saw frame and can be used for cutting a great variety of metallic and non-metallic materials.

When it is desired to armor a flat surface, such as a sheet, and particularly a strip or a plate, a machine of the type illustrated in FIG. 60 can be used to carry the invention into practice. In the present embodiment, a strip 800S is illustrated as being supported and moved by a plurality of rollers 800R. As is obvious to one skilled in the art supplemental driving means may also be used as well as substitute driving means to move the flat surface, such as a steel strip through the machine.

Over the moving strip, a spray or jet 800J is located which applies adhesive, preferably in the liquid or fluid condition, at the adhesive station. After the application of adhesive, powder is distributed across the upper flat surface of the strip at the powder station 800P. A mixture of powders is used which includes a metallic matrix alloy, a diamond substitute or a carbide of a refractory metal and a flux. By allowing the adhesive to dry, the powder is firmly fixed in place on the surface of the strip.

The strip having the powder adhesively affixed thereto is next moved into the induction heating station 800H.

By arranging and shaping an electrical work coil to cover the width of the strip and a selected length, the skin or surface of the steel strip can be heated practically instantly. Controlling the inductive heating permits the control of the heat to a sweating temperature where fusion of the armor occurs and bonding of the armor to the skin or surface of the steel strip is effected.

In the heat treating station 800T, any desired thermal treatment can be effected. Thus, the hot armored strip can first be cooled, chilled or quenched and thereafter subjected to any desirable heat treatment.

As may be seen in FIG. 61, a piece of the armored strip is shown. The armor extends across the entire width and length of the strip. Whenever it is desired, the width of the armor may be controlled. Such an armored strip presents a hard surface which is wear resistant. Likewise, such an armored surface is abrasion resistant. By controlling the amount of diamond substitutes or carbides of refractory metals, the surface may possess an abrading property and/or a cutting property.

Under certain conditions, it is desirable to use a rotary or rotatable machine of a turn-table type or carousel type. In FIGS. 62 to 65, a rotary machine is illustrated which can produce armored articles, tools, component parts and the like in accordance with the present improved induction method of armoring. For example, the armoring of a saw tooth of the type shown in FIGS. 45 to 47 and FIG. 67 can be carried into practice satisfactorily in the rotary machine depicted in FIGS. 62 to 65.

In FIG. 63, a top plan view of a portion of a turn-table 900T is shown. Around the periphery of the turn-table, a plurality of fixtures 900F are mounted at spaced intervals. Each fixture is designed to receive a work piece as may be seen in FIGS. 62 and 63. In the present example, a saw tooth 900S is illustrated as the work piece. As clearly shown in FIG. 62, a selected area 900A to be armored is adjacent to the cutting edge. The selected area includes the corners and adjacent sides.

The adhesive coating containing the powder is applied to the selected area on each saw tooth before it is mounted in a fixture on the turn-table. It has been found convenient to mount each saw tooth manually. Thus, an operator can apply the adhesive coating to the saw tooth and can then mount it in the fixture. By the time the coated saw tooth reaches the induction heating station, the adhesive is dry or is substantially so. In the induction heating station, the coated saw tooth is inductively heated and the skin or surface of the selected area is raised to a sweating temperature where fusion of armor occurs and bonding of the armor to the steel base is effected. Thereafter, the armored tooth will complete its travel during the rest of the cycle. When the armored tooth reaches the terminal station, a kick-off rod 900KO or an operator can remove it. In the event that it is desired to use mass production, each saw tooth may be mounted and removed automatically as is obvious to those skilled in the art. Thus, an unarmored saw tooth is mounted at a starting position and then is removed as an armored saw tooth at a terminal position. Usually, substantially less than 360° of travel is involved. During the travel the saw tooth is inductively heated and is armored. After armoring, the saw tooth is removed.

It is preferred to rotate the turn table by means of an electric motor 900M. While any appropriate driving means may be used, a convenient mode is to couple the electric motor directly to a driving shaft 900D as may be seen in FIG. 62. It has been found preferable to use a pulse motor and related electric circuit as shown in FIG. 65. The use of a pulse motor facilitates the formation of the armor on each saw tooth as it permits inductively heating the selected area for a controlled period of time. A convenient way to provide the control is to have a control gear 900G (see FIG. 64) with a control cam 900C secured in a gear tooth at spaced intervals. It was found that the control cams can be spaced any suitable

number of degrees apart. For illustrative purposes, every sixty degrees is illustrated in the drawings. An arm 900R, for example, is moved by cam 900C (see FIG. 65) and, in turn, moves a contact blade 900K. In its upper position, the contact blade is in engagement with a contact in direct connection with the pulse motor and, in its lower position, the contact blade is in engagement with a contact in direct connection with a timer 900X. This timer is connected with a high frequency generator 900Z which supplies the electricity to an electrical work coil 900W (see FIG. 62). By controlling the period of time during which electricity is supplied to the work coil, the period of inductive heating can be controlled. During this period, there is practically instantaneous heating of the skin and surface of the steel base of the saw tooth where the armor is brought to fusion and where bonding of the armor to the steel base occurs. While FIG. 64 illustrates the mechanical combination, FIG. 65 illustrates the electrical circuit showing the electrical combination.

In practical operations, it was found desirable to make the fixtures 900F of copper. Seated within the copper fixture is a magnet 900MG which holds the saw tooth in its proper position. It is also preferred to shape the upper part of the copper fixture to fit the underside of a part of the saw tooth (see FIG. 62). By so doing, the parts are in close contact and heat can be transferred effectively from the saw tooth to the copper fixture. To make the transfer of heat more effective, the copper fixture may be cooled. For instance, a copper pipe 900P may bring a coolant, such as water, to, through and from the copper fixture as will be well understood by those persons skilled in the art. In this manner, the body of a steel saw tooth is kept cool and heat is withdrawn from the tip of the tooth adjacent to the selected area which is being armored. As soon as the induction heat is discontinued, the cooling of the tooth has a tendency to facilitate a quick solidification of the armor and a bonding of the armor to the steel base. The presence of the copper fixture also has the tendency to concentrate the induction heating on the skin or surface of the steel base of the saw tooth in the region of the tip adjacent to the selected area.

For manual operations, embodiments illustrated in FIGS. 66 to 68 have been found to give satisfactory service. Thus, the embodiment shown in FIG. 66 functioned satisfactorily for the armoring of sickle sections depicted in the drawings and particularly in such figures as FIGS. 2, 7, 8, 9, 21, and 22. A selected area of a sickle section or blade 1200S adjacent to its cutting edge is adhesively covered with powder and is dried. It is mounted in a bracket 1200B which is pivoted in a supporting arm 1200A. Such pivoting permits the bracket to be manually operated by an operator. By moving the bracket toward an electrical work coil 1200W, the coated sickle section can be moved into a proper position within the work coil to enable it to be inductively heated and to cause the armor to be fused and to be bonded to the steel base. After induction heating, which is practically instantaneous, the bracket is swung away from the work coil and the armored sickle section is removed in an appropriate manner. This armored sickle section will be similar to those armored in the machines illustrated in FIGS. 14 to 35 and FIGS. 37 to 42C.

In the event that it is desired to armor a saw tooth such as shown in FIGS. 10 to 12 and 45 to 48 or to armor a chip breaker of the types shown in FIGS. 49 and 50, embodiments shown in FIGS. 67 and 68 may be used. In both illustrations, the work pieces are first adhesively coated with powder and dried before subjecting them to induction heat. In FIG. 67, a bracket 1200K may be moved in and out manually. Upon the bracket, a fixture 1200F is mounted which carries a saw tooth 1200T. By moving the bracket inwardly, the saw tooth is brought into the proper position within an electrical work coil 1200X where armoring is effected. After armoring, the bracket is moved outwardly where the armored

saw tooth may be removed and may be replaced with another saw tooth which is to be armored. A chip breaker can be armored in the same manner, except a modified form of bracket is employed. By referring to FIG. 68, it will be seen that a bracket 1200R is a pivoted type and carries a fixture 1200U. The bracket may be pivoted in and out and the chip breaker can be armored by moving it within an electrical work coil 1200X. When the bracket is moved to its outward position, the armored chip breaker can be removed and can be replaced with one to be armored.

Still another embodiment of the invention can be used when an edge is to be armored. For instance, when the edge of a strip or plate is to be armored, the arrangement and combination illustrated in FIG. 69 can be used. A supporting base 1300B is provided over which a strip 1300S can slide. For guiding and moving the strip along the base, a plurality of rolls 1300R can be utilized which are in frictional engagement with the side of the strip.

As the strip is moved along, it passes the various stations where the essential operations are conducted. Adhesive is applied at the adhesive station to the edge of the strip by means of a porous roll 1300P. The adhesively coated strip proceeds to the powdering station where powder is sprinkled onto the coated edge by suitable means, such as a magnetic feeder or a vibrator 1300V or the like. By the time the powdered strip reaches the induction heating station, the adhesive is dry or practically so. When desired, a drying station can be placed between the powdering station and the induction heating station.

To inductively heat the adhesively coated and powdered strip, an electrical work coil 1300W is provided at the induction heating station. By controlling the heat, a sweating temperature can be produced where fusion of the armor occurs and bonding of the armor to the steel base takes place. Under certain conditions, it is sometimes preferable to provide a supplemental rod 1300O. The tip or end of the rod melts and flows into the armor and becomes a part thereof. As those persons skilled in the art will understand, the rod may have any desirable composition. Thus, it may have a ferrous or steel base harmonizing with the ferrous or steel base constituting the strip or it may have a tungsten, cobalt or other base harmonizing with the metallic matrix alloy or some other composition compatible with the metallic base of the strip, the metallic matrix alloy and the diamond substitute, such as carbide of tungsten and the like.

The armored strip can be used in suitable lengths. It can be utilized in a length which fits tools for manual operation or in a length which fits machines for automatic operation. In either case, the armored edge can be used to cut metallic and/or non-metallic materials. Due to the hardness of the armored edge, it is also wear resistant.

When a rotatable article is to be armored, such as a rotatable feed screw 1400S, the arrangement illustrated in FIG. 70 is found to be satisfactory. In the arrangement shown in FIG. 70, the rotatable feed screw 1400S is mounted in a lathe which can rotate it at a controlled number of revolutions per minute as will be understood by those skilled in the art. As a result of use of rotatable feed screws in extrusion machines for feeding plastics and the like, it was found that the outer edge of the blade was subject to wear. It was found desirable to armor an outer edge 1400E and adjacent sides 1400A of a helical blade 1400H of the feed screw. When thick armor is desired, a supplemental rod may conveniently be used. For example, it is preferred to use a Stellite rod.

In practice, the feed screw can be moved horizontally or can be stationary as shown in FIG. 70. In either case, those persons skilled in the art will appreciate that the feed screw must be rotated at a very slow rate to permit armoring of the selected area comprising the outer edge and adjacent sides of the helical blade. The selected area is adhesively coated and powdered while rotating the

feed screw in the lathe. The powdered coating is dried in any convenient manner. Infrared heat lamps may be used conveniently for the drying operation.

In order to inductively heat the selected area to be armored, a suitably shaped electrical work coil 1400W is arranged about the outer edge of the helical blade of the feed screw. An enlarged detail view of the arrangement is illustrated in FIG. 71. High frequency electricity is supplied to the work coil by an appropriate electrical auxiliary including a transformer 1400T. For convenience, the electrical auxiliary is carried upon a movable platform 1400P. This platform moves on a pair of slides 1400L of well known construction. Likewise, a suitable jack screw 1400J moves the platform in a proper direction and at the proper speed. The movement of the jack screw is coordinated with the rotation of the feed screw as those persons skilled in the art will understand. Thus, the armoring begins at the right-hand end of the feed screw and proceeds to the left-hand end. As the selected area on the helical blade is armored during rotation of the feed screw, the platform is moved gradually from the right-hand side of the lathe to the left-hand end. In this manner, the entire outer edge and adjacent sides of the helical blade can be armored.

An alternative embodiment is illustrated in FIG. 72. In this embodiment, the electrical work coil 1400W is held stationary and the feed screw 1400S is moved horizontally while at the same time it is rotated. The armoring is conducted in the same manner as described hereinbefore.

To facilitate the armoring and to improve the control of the induction heating, auxiliaries or supplemental machines are employed. Thus, as a result of tests, it was discovered that armoring could be conducted under optimum conditions by using a temperature sensing device. As is well known in the art, alternating electric current is delivered by public utilities to shops, laboratories and factories using electricity. Due to the fluctuating use of electricity by users, there is a fluctuation in the line voltage at the user's premises and at the user's machines and equipment. Such fluctuations cause fluctuations in the voltage and current delivered by the high frequency induction generator which provides the high frequency alternating current used by the electrical work coil. Fluctuations in this work coil cause other fluctuations in heat in the work piece, such as the outer edge of the helical blade of the feed screw. Other variables include a movement of coil, changes in the root diameter of the feed screw and the like.

By providing a temperature sensing device 1400D above the work piece as may be seen in FIG. 72, it may be focused on the area undergoing induction heating. Whenever the heat fluctuates or changes in the area, the temperature will fluctuate or change. Such temperature change will affect the temperature sensing device which in turn will affect the electrical control system to the induction generator and output transformer as clearly shown in FIG. 72. It was discovered that the best combination in an electrical control system is a feed back controller combined with a saturable reactor. Although a saturable reactor is preferred, a power manipulator may be used in its place. This combination controls the electrical energy coming from the induction generator and output transformer and going to the electrical work coil. With this control system, the electrical energy can be controlled as well as the temperature in the area of the work piece undergoing armoring. As a result of this control, the armoring can be facilitated and controlled.

For armoring thin disc-like articles, such as a rotary or rotating cutting device like a disc cutter, arrangements and combinations such as illustrated in FIGS. 73 to 77 have been satisfactory. While any appropriate combination may be used to carry the invention into practice for armoring thin disc-like articles, the machine shown in FIG. 73 was found to be convenient. A T-shaped frame

1500F is mounted on a main pivot 1500P. At approximately the center, a stub shaft 1500S is provided for mounting a disc cutter 1500D. To assist in cooling the disc cutter during the armoring operation, a cooling chamber 1500C is provided at the end of the vertical arm of the T-shaped frame. This chamber is in contact with the rear face of the disc cutter as those persons skilled in the art will understand. For the purpose of providing cooling on the front face of the disc cutter, a second cooling chamber 1500K is mounted on a swinging bracket 1500B. It is preferred to mount the second cooling chamber in a resilient manner, such as by use of a pair of springs 1500R. When the swinging bracket is rotated about a shaft 1500E depending from the T-shaped frame near the main pivot, the second cooling chamber can be moved into contact with the front face of the disc cutter. In this manner, one cooling chamber covers an area on the disc cutter's rear face while an approximately corresponding area of the front face is covered by the second cooling chamber.

The armoring operation is conducted by tilting the T-shaped frame about the main pivot and moving it downwardly a few degrees. By so doing, a segment 1500G on the periphery of the disc cutter between adjacent slots 1500L can be brought within an electrical work coil 1500W. The tilting movement is effected by the use of an air cylinder 1500A which is operatively associated with the free end of the right-hand arm of the T-shaped frame. After armoring a narrow band 1500N on the segment, the T-shaped frame and the mounted disc cutter can be tilted back to its normal position. The disc cutter can be rotated a few degrees to its next position for armoring another segment. The frame is again tilted and the new segment brought within the electrical work coil to armor another narrow band. The foregoing operations are repeated until all of the segments are armored. As an alternative mode of procedure, the frame can be held in its downward tilted position and the disc cutter rotated a few degrees to move a new segment in an armoring position. Of course, the high frequency electric current is turned off during each rotation and is turned on again when the new segment is in its armoring position.

For certain uses, the peripheral edges of the segments are covered with cutting diamonds. As is well known in the art, the cutting diamonds are held in molded pieces which can be silver soldered to the edges. The armored sides not only provide hard, wear-resistant bands but also provide cutting faces. When a disc cutter is used for cutting cementitious materials like concrete, cement and the like, the cut material has to be disposed of. To assist in the disposal, a circular gullet 1500U is merged with the inner end of each slot 1500L.

When the peripheral edge 1500I of a disc cutter is to be armored, the arrangement illustrated in FIG. 74 can be used. By rotating the disc cutter a few degrees about the stub shaft, the peripheral edge of each segment can be armored. In this manner, the entire peripheral edge can be armored. The armored disc cutter can be used for cutting various metallic and non-metallic materials.

In armoring disc cutters and the like, it was found that a special transformer of novel construction produced improved results. The novel construction is clearly shown in FIGS. 74 to 76. A primary 1500PR of a transformer has a plurality of turns closely wound in the form of spiral. The close winding may be clearly seen in FIGS. 74 and 75. Closely adjacent to the primary is a secondary 1500SC of the transformer. For best results, the secondary comprises a single coil which is preferably rectangular in cross section (see FIG. 75). A lead-in conductor 1500LC is fastened to a vertical partition 1500VP of a high frequency (H.F.) induction generator system and is connected to the inner end of the spirally wound primary whereas a second lead-in conductor 1500LK is fastened to a second vertical partition 1500VQ and is connected to the outer end of the spirally wound primary

by means of a weld 1500WE. The weld may be clearly seen in FIG. 76. Partition 1500VQ is electrically connected to a ground 1500GR.

Below the weld, the end of the outer coil of the spirally wound primary is connected to one end of the single coil of the secondary. The other end of the primary is connected to one end of the electrical work coil 1500W (see FIG. 74). The second end of the work coil is connected to the second lead-in conductor 1500LK.

For best results, it was found that hollow copper tubing should be used for the entire transformer and work coil combination. By using the illustrated arrangement, a series flow of cooling water may be maintained throughout the system. In this manner, a stream of water or other coolant may be sent through the series connected copper tubes under high velocity to insure rapid heat transfer from the inner walls of the tubes to the stream of water or coolant. The temperature in the tubes may be controlled to some degrees within a selected safe range. Consequently, the difficulties and disadvantages of the conventional parallel system of cooling are avoided. This is especially true of over-heating in one coil, especially at dangerously high temperatures.

The compactness of the transformer is clearly depicted in the figures and particularly by FIG. 75. This compact arrangement makes it possible to have it connected electrically directly to the work coil without the necessity of using the conventional long leads. Those persons skilled in the art will appreciate that the novel combination can effect a great saving in electricity by eliminating the usual electrical losses in the long leads. Likewise, the new arrangement will be safer with the elimination of long leads. A further safety factor is the grounding of the system.

The novel electrical circuit is shown diagrammatically in FIG. 77. The high frequency (H.F.) induction generator is clearly illustrated and is connected to the primary 1500PR of the transformer. Closely associated with the primary is the secondary 1500SC of the transformer. The secondary is directly connected to the electrical work coil 1500W. Between the primary and secondary, a branch of the circuit constituted by a lead-in conductor is grounded by a ground 1500GR.

In the event that it is desired to armor a bar of rod 1600B provided with a plurality of teeth 1600T, the combination shown in FIGS. 78 to 81 can be used. The combination is similar to the one illustrated in FIGS. 74 to 77. A primary 1600PR of a transformer is constituted of a plurality of coils in a tightly wound spiral and a secondary 1600SC is constituted of a single coil (see FIG. 79). It is preferred to make the primary of circular copper tubing and the secondary of square copper tubing. A lead-in conductor 1600LC constituted of circular copper tubing is connected to the inner end of the spiral tubing of the primary whereas a second lead-in conductor 1600LK constituted of circular copper tubing is joined to the outermost coil of the primary by means of a weld 1600WE (see FIGS. 79 and 80). One vertical partition 1600VP is fastened to lead-in conductor 1600LC by any convenient means, such as welding. A second vertical partition 1600VQ is fastened to the second lead-in conductor 1600LK by welding or the like. This second partition is grounded by ground 1600GR.

Due to the compact arrangement, the transformer may be connected directly to an electrical work coil 1600W without the necessity of using conventional long lead-in conductors. The armoring operations are similar to those in connection with the circular cutter disc described in connection with FIGS. 73 to 77. However, the bar 1600B may be moved continuously at controlled speeds to permit continuous armoring. Depending upon the desired product or mode of production, either step-by-step armoring or continuous armoring may be used.

The electrical circuit illustrated in FIG. 81 is similar to the one shown in FIG. 77. A high frequency (H.F.) induction generator is connected directly to a primary

1600PR of a transformer. The secondary 1600SC is connected directly to an electrical work coil 1600W. A branch of the circuit going from the junction of the primary and secondary to the generator is grounded by means of a ground 1600GR. The electrical and other operations are the same as those involved in FIG. 77. It has been found that the circuit including the compact combined transformer and inductor or work coil has many advantages including electrical efficiency and economy, shortness of leads, safety, and close coupling to the work thereby permitting better control of the heat pattern. The secondary of the output transformer is a single turn and the work coil is itself only a simple short loop. Thus, there is a relatively low voltage across these components, although the current they carry is high. Further, the point of common connection of the primary and secondary of the output transformer and the return connection from the work coil is grounded. As a result, no part of the work coil or of the secondary of the output transformer is very far above ground potential. This is an important advantage for with close coupling any great potential difference would tend to cause arc over to the work piece which is preferably maintained at ground potential. Such tendency to arc over is aggravated during periods of high humidity or by the emission of smoke or ionizable gases as temporary adhesives and/or fluxes are heated in the coil. Not only will an arc-over be a safety hazard to operators who may be in contact with other parts of the machine but it will usually throw out the circuit breakers in the induction generator and interrupt the operation thereof. Another advantage is the compactness of the combined transformer and inductor or work coil. Due to the compactness, all of the extensions of or from long leads and the like are eliminated and the high frequency can be maintained. Likewise, space radiation tends to decrease with compactness. As is well known, any extra length of leads, extension and the like in the tank circuit affects the frequency of the system which is eliminated by the compact combined transformer-inductor. When long leads of the prior art are used, losses are encountered and such losses require higher voltages across the primary in order to get enough energy to do the armoring in the work coil. It is also known that the tank circuit must be of the least geometry in order to maintain the desired high frequency. Since the new combined transformer-inductor is so compact, the maintenance of the desired high frequency is facilitated.

The present invention provides an improved induction method for armoring a metallic tool having a selected area to be armored which comprises coating the entire surface of the area to be armored with an adhesive composition decomposable by heat and of a consistency such that it covers the said area with a film of adhesive that retains the exact configuration of the surface of the area which it covers, powdering the applied adhesive with a fine powder comprising a refractory armor material which adheres to the adhesive in a thin layer conforming precisely to the configuration of the surface beneath the adhesive, said armor material having a relatively high range of fusion and having the property when fusing of bonding with said surface of the tool, and inductively heating the powdered surface to cause practically instantaneous decomposition of the adhesive and fusion of the powder directly upon the underlying surface evenly in a surface-bonded layer of refractory armor replacing the adhesive and thereby, to the same degree as the adhesive, retaining the configuration of the underlying surface of the tool, whereby an improved armored metallic tool is provided.

It is likewise within the contemplation of the present invention to provide an improved induction method of armoring which is especially useful for making armored cutting tools. Such armored cutting tools embrace a large variety and include those disclosed herein and illustrated in the drawings. Some of these armored cutting

70  
75

tools may, for illustrative purposes, include armored reciprocating saw blades, band saw blades, circular saw blades, files, rasps, sanding screens and disks, abrasive sheets, core drills, and the like. An outstanding characteristic of these refractory armored cutting tools is the presence of a myriad of relatively small individual cutting teeth provided by exposed sharp edges of hard, refractory particles of diamond substitute materials, such as tungsten carbide, projecting from the surface of the refractory armor. In each case, the hard, refractory cutting particles are embedded in a refractory matrix alloy which is tenaciously bonded to a metallic base of the cutting tool which is usually made of steel for practical and industrial tools. The matrix is constituted of a hard refractory alloy capable of wetting the surface of and bonding to the hard refractory cutting carbide particles and also capable of alloying by fusion with and/or diffusion into the surface layer or skin of the underlying metallic base of the cutting tool. When the refractory alloy is one which undergoes fusion only at a relatively high range of temperatures well above the upper transformation point of the metallic steel base, that base can be heat treated by any conventional procedure to develop any desired combination of strength, hardness, toughness and ductility, without affecting the ability of the matrix alloy to tenaciously retain the cutting carbide particles. Suitable matrix alloys may be those disclosed in my Patents No. 3,023,490 and No. 3,024,128 or in my co-pending application referred to herein. In much of my experiments, tests and operations, I have preferred to use an alloy of cobalt, chromium and tungsten, such as an alloy sold in the market and under the trademark Stellite or one which is identified as No. 33W by its manufacturer, the Crucible Steel Company, which sells it to the trade. It likewise has been found preferable to use a nickel base alloy with chromium, boron and silicon, such as Haynes "43-C" alloy or Colmonoy "Nicrobraz" alloy "LM."

Illustrative of armored cutting tools is a wire saw possessing unusual cutting characteristics and adopted for use in a conventional hacksaw frame or similar reciprocating saw. Such a saw is preferably made of an alloy steel wire of about 0.070 of an inch in diameter. It may be secured at its ends by washers or eyelets. (See FIGS. 57 to 59). They are secured to the ends by any appropriate means, such as spot welding, silver soldering, or the like.

The armored steel wire may then be heat treated by any appropriate or conventional methods, such as heating above the transformation, then quenching, and subsequently tempering in order to secure the desired combination of toughness, hardness, strength and ductility. After the heat treatment, the armored steel wire may be used as is, or it may be rendered more attractive for commercial sale by lightly plating with a white metal, such as cadmium, or by painting with a light colored paint.

It has been found that such an armored steel saw is extremely effective in cutting materials which cannot be cut at all by ordinary techniques or can be cut only with difficulty. For example, such a saw will readily cut glass, ceramics, stone, brick, hardened tool steel, stainless steel, titanium, hard and refractory alloys, etc. It is with such materials that the present invention finds its greatest utility. Since such an armored steel saw is in wire form, it can cut in any direction to form intricate curves, and, since it cuts on both the pushing and pulling strokes, it is fast and relatively easy to use. The hard, refractory carbide particles constituting the cutting teeth are so tenaciously bonded that they will not separate or pull off in use and the steel wire may be flexed and bent without disturbing the bond.

The size and type of cutting particles to be used can obviously be widely varied to suit the requirements of specific jobs, as those persons skilled in the art will appreciate. For example, a relatively fine granulation of

tungsten carbide particles (e.g. 60/100 mesh) is best adapted to cutting glass and glass-like or glazed surface materials, such as ceramic tile, to minimize spalling and chipping of the brittle material. Similarly, for faster cutting of any material or for cutting wood and certain plastic materials, relatively coarser teeth should be provided as by the use of larger particles (e.g. 40/60 mesh) in sparse distribution. A good general purpose saw is provided by the use of carbide particles of about 50/70 mesh granulation, such as those sold on the market by Kenna Metal, secured by a matrix of "Crucible 33W" cobalt, chromium, tungsten and boron alloy or by a nickel base alloy with chromium, boron and silicon, such as Haynes "43-C" alloy or Colmonoy "Nicrobraz" alloy "LM," to a No. 4037 steel wire having a diameter of about 0.070". It is preferred to heat treat such a steel wire to develop maximum strength consistent with maintaining sufficient flexibility to avoid breakage as a result of the unavoidable flexing in use. The cemented carbides are preferably to the cast carbides which on crushing to produce small fragments tend to shatter into needle-like splinters which are not well adapted to serve the purposes of the present invention. Chunks or nodular particles of the cemented carbides of size appropriate to the particular application and fairly uniformly of that size are preferable.

Depending on price and availability, the carbides of any of the refractory metals or their mixtures may be used satisfactorily. For example, the carbides of silicon, tungsten, molybdenum, chromium, tantalum, niobium, vanadium, titanium, zirconium, and boron, may be used, although carbide of tungsten is preferred by virtue of its wider availability.

The present invention is not to be confused with old inventions in the prior art. Thus, an alloy rod interdispersed with diamond-substitute granules or a tube rod filled with diamond-substitute granules was used by holding above the surface to be coated and a molten mass flowed on by means of heat, such as provided by a torch or electric arc. (See, for example, U.S. Patents Nos. 1,650,905; 1,757,601; 1,803,875; and 2,033,594.) This prior method lacked control of thickness of surface and distribution of diamond substitute granules. It could not precisely follow the contour of the surface. This was particularly true where unprotected square corners were rounded and melted off due to the difficulty of controlling the heat of the welding torch. Ripple marks were likewise left on the surface when hand welding with an electric torch was used. When working from a rod or tube with a torch, it was practically impossible to melt an even amount from the supply end of the rod and spread it uniformly over several different unit areas in the thinness tolerance contemplated by the present invention. In fact, the degree of precision involved in producing a uniform surface on the novel armored metal article was so much greater than that made, intended or required for use by the old tube method that this old method is entirely different from the present improved method of armoring. When it became necessary to smooth the surface as by grinding, the best part of the coating was ground away. Another method involved the distribution of refractory grains or particles onto a molten surface. (See for example, U.S. Patent No. 1,733,241.) The surface to be coated was molten until a very thin layer of the base metal became molten. Before this molten surface had an objectionable amount of oxides formed, the diamond substitute granules were distributed or dispersed over the molten area. They sank in and caused the base metal to be bonded thereto. With this old molten method, the conditions under which the distribution was done required so much skill that it was very costly for industrial production and that it could only be used for very special situations. It was practically impossible in a convenient manner to do the underside of an article and very difficult to do the sides. Minute contours were almost impossible to follow, especially

sharp corners, thin projections, etc. Still another prior method involved coating a surface with refractory grains and then heating it very rapidly to produce tungsten carbide in situ on the surface of the base metal, such as steel. (See, for example, U.S. Patent No. 1,824,166.) 5 Tungsten or a tungsten-containing material was mixed with carbon and applied to the surface with an adhesive. By use of some method of high heat, such as by an arc, the tungsten-containing material was reduced by the carbon and tungsten functions like finely divided tungsten and reacted with carbon to form tungsten carbide in situ which sank into the molten surface of the base metal caused by the application of the heat. In general, it took an appreciable time and/or excessively high temperature above the melting point of the steel constituting the ferrous tool to form tungsten carbide in situ in appreciable quantities. If the temperature were raised above the melting point of the steel, it would obviously be impossible to reproduce the contour of the part with accuracy. Any attempt to 10 use the excessively high temperature required would need an atomic hydrogen arc which would inevitably melt the sharp cutting edges to be armored. These operations were difficult to carry into practice on an industrial scale for 15 commercial production. Another disadvantage of these operations was that they produced a very uneven coating, 20 burnt off sharp edges, etc. A further prior method involved electroplating of chrome on the surface of the metal article. The chrome was merely for the purpose of prolonging the life of a tool. However, the chrome-plated 25 article did not hold an edge and the coat was not thick enough to provide strength required for a built-up edge 30 to form when the steel wore away. Other metals used for plating or coating were aluminum, bismuth, cadmium, 35 cobalt, copper, nickel, tin, zinc and the like. Glass and glazes have been proposed, but such brittle materials 40 have no strength and crack, spall, split, shatter, etc., from the surface. A still further prior method involved metal spraying. In metal spraying, no fusion bond was formed. 45 The bond was merely mechanical and did not possess the strength and the properties required for practical operations. It would be difficult to get a uniform coating on an irregular shaped piece. Even on a simple shape as 50 a saw bit having three sides, it would be difficult without expensive mechanical aids to coat the three surfaces with the same thickness. It would be practically impossible to treat an interior surface having only a small opening. For 55 example, it would be difficult to treat a hollow drill with a hole of an appropriate diameter, such as  $\frac{1}{4}$ " or  $\frac{3}{8}$ " or so. On the other hand, if such a hole, slot, etc., has such a diameter as to permit an end of a coil or a loop 60 thereof to be placed inside of the hole, slot, etc., then the interior can be armored by the present invention. The prior art also used briquetted and sintered pieces or 65 inserts and sold them under such trade names as Carboloy. The inserts were brazed to tools. Attempts were also made to mechanically fasten particles of tungsten carbide to a metallic base, such as a steel article. The disadvantages 70 were: first, high cost due to the larger amount of expensive material and the greater labor required to make and install them; and second, the thicker insert was not self-sharpening. When re-sharpening was necessary, it was much easier to work the present armored article. Although grinding was preferred, the present armored articles can be filed to sharpen them. This is made possible by the extremely thin coating made by the present invention. The prior inserts brazed to tools might be used only under very special conditions. Other methods used heretofore attempted to use varnish, lacquers, etc., and metal powders for decorative purposes on sheet material, such as paper, cardboard, plastic and the like. If 75 heated to a high temperature or brought into contact with hot things—especially red hot or white hot—the paper, etc., would go on fire or would scorch or otherwise be destroyed or made useless.

In contrast with the prior art, the present invention

provides an improved induction method of armoring a selected surface of a metal article with a thin, flat, refractory, hard-wearing, abrasive, cutting surface of smooth and uniform character and of uniform thinness containing hard sharp particles of a diamond substitute and conforming to the exact contour of the selected surface. The refractory armor or hard facing comprises a hard refractory matrix, such as Stellite, martensitic iron, nickel boride or equivalent, containing hard refractory or diamond substitute particles, such as tungsten carbide or the like. The coat of refractory armor is extremely thin, such as about 0.002" to about 0.005". In exceptional cases, the coat can have thinnesses up to about 0.015". The thin coating of refractory armor accurately reproduces the underlying contour including irregularities, square corners, etc. All prior coats made the corners round. The new invention contemplates the provision of an adhesive composition which tends to cover and to flow evenly over the article or work piece being armored and to form a thin film on the selected area. Such a film retains a uniform thinness of metal powder comprising matrix alloy and hard refractory particles when the powder is dusted or sprinkled over the article or piece. Most prior hard-facing processes fail to provide means for obtaining a uniform thickness. Consequently, the prior processes cannot be used where accurate reproduction of a contour is to be effected.

Armor can be applied to internal slots, holes, etc., by the present invention whereas prior processes requiring a torch or electrode for heating could not be used for such purposes. On cutting tools, the improved method applies hard refractory armor to the clearance sides instead of on the cutting face as is effected by most prior hard-facing processes. The armoring of the clearance sides allows the tool to be sharpened many times without removing the armor. By armoring the clearance sides only, wear on the cutting face of the tool sharpens the cutting edge of the armor. Such clearance side armoring of tools makes it much easier to sharpen them as the amount of carbide to remove is relatively small due to the thinness of the armor coating. The extremely thin coat of refractory armor applied by the present invention makes it possible to restore the corner of a tool by swaging. This is impossible with thicker coats of armor applied by prior processes.

Although the present invention has been described in conjunction with preferred embodiments, it is to be understood that modifications and variations may be resorted to without departing from the spirit and scope of the invention, as those skilled in the art will readily understand. For instance, instead of a ferrous base for the metal article, tool, component part or work piece, non-ferrous bases can be used, such as copper bases (brasses, bronzes, etc.) or nickel bases or cobalt bases or molybdenum bases or the like. Likewise, the metallic matrix alloy may be constituted wholly or partially by other suitable alloys, such as cobalt alloys, nickel alloys, iron alloys—particularly or austenitic or martensitic character, and the like. However, generally speaking, tungsten alloys have given satisfactory service and particularly tungsten-cobalt base alloys or tungsten-cobalt-chromium base alloys and especially those of the type sold in the market under the brand name of Stellite. For special purposes, cobalt alloys and/or nickel alloys have produced satisfactory results. Instead of the shellac solution, other suitable organic adhesive or binder materials can be used. For example, appropriate solutions containing natural or synthetic rosins and/or resins, such as glyptals, silicones, phenol-formaldehyde resins of the Bakelite type, cycopolys (sold by Oliver Johnston Paint Company). Varnish, lacquer or Tung oil may be used. Other water or alcohol solutions may likewise be substituted, such as solutions of sodium silicate, etc. Instead of borax, other flux materials may be employed, such as borate-containing materials, boric acid, sodium or potassium fluoborate,

sodium or potassium fluoride, sodium silicate, lithium salts such as fluoride, metaborate or tetraborate, and the like. As those skilled in the art know, the melting points of these fluxes vary up to about 1,500° F. to about 2,000° F. Similarly, the operations can be varied. Thus, the metal powders and fluxes can be added to the solution of adhesive or binder and thereafter an appropriate operation, such as dipping, brushing, spraying or painting the adhesive or binder solution on the entire or selected area can be used. Subsequently, an operation can be employed to evaporate the solution and thus form a dried coating on the article, tool, component part, or other work piece. Finally, the surface can be inductively heated to fuse the armor coating to metal base. On the other hand, the surface to be armored can be painted or printed with binder or adhesive and then can be powdered with refractory particles of diamond substitutes, such as tungsten carbide by sprinkling such particles onto the film of adhesive. Thereafter, powdered material including a metallic matrix alloy, such as Stellite, a flux such as borax, and optionally a carbohydrate can be sprinkled over the surface to surround the particles of diamond substitutes. Another variant is to sprinkle all powdered materials on together. On the other hand, the powdered materials can also be put on the adhesive film on the article separately. For instance, the diamond substitute can be applied first, the matrix alloy second, and the flux third. The order can be varied by putting the powder comprising the matrix alloy on first, next the diamond substitute particles can be put on, and finally the powdered flux can be sprinkled on. When all of the powdered material is to be applied together to or sprinkled over the adhesive coating or film, care must be taken to avoid segregation or stratification of materials of such widely differing density as tungsten carbide and flux, as those skilled in the art will readily understand. To avoid such segregation and stratification the powders are preferably blended in a powder blender. As those skilled in the art know, a powder blender is a tumbling device of "Y" shaped configuration rotated about an axis perpendicular to the straight arm of the "Y" and passing through both of the double arms of the "Y" near their point of intersection with the single arm. As the device is rotated, the powder is lifted in the single arm and dumped to fall and divide more or less equally between the other two arms. When they in turn are dumped, the two streams of powder converge and fall together into the single arm. Such blenders are in common use and are well known in the art for blending all sorts of powdered or granular material.

When powdered materials are so blended, they are mixed with a shellac solution until the powders are evenly wet with shellac and have a consistency about of moist sand. The powder so moistened is spread out into a thin layer and scored to define a plurality of small rectangular wafers or briquettes. After these wafers or briquettes are almost thoroughly dry, they are crushed in any conventional small mill to provide a coarse powder in which each individual granule is a uniform powder mixture of matrix alloy, diamond substitute and flux bonded together with a small amount of shellac or other temporary adhesives of the types described herein as compatible with the novel improved method. When powders are so treated, they will not segregate or stratify to any substantial extent when fed through a vibratory feeder since even the fines resulting from the crushing operation are mixtures held together by the shellac or other adhesive. If dry powders are used without such a bonding operation in vibratory feeders, it is desirable to take special precautions to minimize segregation. For example, a vibratory feeder may be modified by the provision of a feed funnel which terminates slightly above the bottom of the inclined vibrating chute of a vibratory feeder. Powder placed in the funnel will feed out in a thin layer on the bottom of the vibratory feed chute and if the excess powder delivered by the chute is continually or intermit-

tently fed back into the funnel the powders reblend and segregation of constituents is at least minimized. Of course, various other combinations can be used including the application of several coats with or without additional films or layers of adhesive. The coated metal article can be dried and then subjected to induction heating to fuse the matrix and bond the armor coating to the metal base. Heating can be accompanied, if desired, with a controlled atmosphere, such as dissociated ammonia, argon, or other neutral or reducing gas. The latter heating operation can be varied by adding methane ( $\text{CH}_4$ ) or natural gas to the controlled atmosphere, such as dissociated ammonia. Various frequencies can be used in the induction heating. Generally speaking, the selected frequency depends upon the particular conditions and especially the size of the work piece. As a general rule, the lower the frequency, the deeper the skin effect and, on the other hand, the higher the frequency, the thinner the skin effect. Usually, a sufficiently high frequency is selected to overcome any cancellation of the skin effect as is well known to those skilled in the art. As a result of experiments and tests as well as practical operations, a preferred range of frequencies, which have been found to be satisfactory, extends from about 300 or 400 kilocycles to about 4 or 8 megacycles. The former frequencies have been found to give satisfactory services for thicker work pieces whereas the latter frequencies produced satisfactory results with thinner work pieces. The high frequency electric current can be brought to an electrical work coil in any suitable manner, such as the conventional long leads, but whenever it is appropriate, it is preferred to use the compact combined transformer-inductor described herein and illustrated in the drawings. Such modifications and variations are considered to be within the purview and scope of the invention and appended claims.

I claim:

1. In an armoring method of applying to a selected portion of a surface of a metal article, a hard armored surface conforming to the shape of the metal article by a combination of operations including wetting the selected portion of the surface with a liquid binder composition having the property of decomposing as an incident of the method and of a consistency such that it spreads evenly and at a substantially uniform thickness over such selected surface upon contact therewith, coating the wetted surface with powdered armor material so that it adheres readily thereto in a layer having the contour of the surface, said powdered armor material comprising powdered hard refractory metallic matrix alloy and powdered diamond substitute particles and having at least a part of the powdered armor material possessing the property when melted of bonding with the surface of the metal article, and subsequently raising the temperature of the surface of the metal article to a fusion bonding temperature to remove the wetting composition and to effect fusion bonding of the powdered metallic matrix alloy onto the selected surface of the metal article in a self-conforming fused layer with the powdered diamond substitute particles dispersed and bonded therein, the improvement which comprises the steps of concentrating on the surface of the selected portion of the coated article intense induction heat produced by alternating electric current having a sufficiently high frequency of at least several hundred kilocycles to increase the temperature practically instantly within the skin of the metallic surface of the metal article to the sweating point and to cause heat to flow outwardly from the said metallic surface to and through the coating of armor material, controlling said induction heating for a short momentary period of time of not more than a fraction of a minute and sufficient to produce a sweating temperature and to cause bonding of the metal article to a coat of armor comprising hard refractory metallic matrix alloy containing dispersed diamond substitute particles, and discontinuing said induction heating immediately after the sweat-

ing point has been reached and after a unitary refractory metallic coat of armor has been bonded to the metallic surface of the metal article whereby practically instantaneous solidification of the hard refractory metallic armor coat on the metal article is effected, whereby a coat of armor is formed only on the surface of the selected portion of the metal article conforming to the contour thereof, and whereby the hard refractory metallic matrix alloy of the armor coat and the metallic surface of the metal article are fused together with an interfacial metallic bonding layer.

2. In an armoring method of applying to a selected portion of a surface of a ferrous article a hard armored surface conforming to the shape of the ferrous article by a combination of operations including covering the selected portion of the surface with a thin film of a binder material having a consistency such that it coats evenly all parts of the selected surface and having a composition such that it adheres thereto, is chemically inert to the material of the surface and to pulverulent material of the armor, is compatible with all operating conditions of the process, and dissipates as an incident thereof, applying to the film of binder a coating of pulverulent armor material comprising a hard refractory metallic matrix-forming material and powdered diamond substitute particles, and subsequently heating the powder-coated article to dissipate the binder and melt the matrix material so that it bonds to said coated surface and to the diamond substitute particles forming therewith a hard armored surface exactly reproducing the entire selected portion and contour of the underlying surface of the ferrous article, the improvement which comprises the steps of restricting intense electrical inductive heat produced by alternating electric current having a sufficiently high frequency within a range of about 300 kilocycles to about 8 megacycles on the surface of the selected portion of the ferrous article to effect a practically instantaneous heating of the skin of the metallic surface of the ferrous article to a sweating temperature and to cause heat to flow outwardly from said metallic surface to and through the pulverulent armor material, and only continuing said electrical inductive heat for a momentary period of time of about a few seconds to continue the outward flow of heat to effect a practically instantaneous fusion of the pulverulent armor material together and to the underlying surface of the selected portion of the ferrous article to be armored whereby a ferrous article is produced having a controlled coat of hard armor, a firm controlled penetration of the armor material into the surface of the selected portion of the ferrous article to form a tenacious bond between the surface of the ferrous article and the coat of hard refractory armor, and an effective retentio by fusing particles of diamond substitutes within the coat of hard armor and whereby effectiveness of the abrasiveness, sharpness, and hardness of the hard armor coat continues in service.

3. In an armoring method of applying to a selected portion of a surface of a ferrous tool a hard armored surface conforming to the shape of the ferrous tool by a combination of operations including coating the selected portion of the surface of the ferrous tool with an adhesive binder and pulverulent armor material containing a hard refractory metallic matrix, a fusible flux having adhesive properties when fused, and a carbide selected from the group consisting of the carbides of silicon, tungsten, molybdenum, chromium, tantalum, niobium, vanadium, titanium, zirconium, and boron, and subsequently heating the coated ferrous tool surface at a temperature and for a period of time sufficient to reach the sweating point of the base metal of the ferrous tool whereupon there is a fusion of the matrix of the surface layer of the ferrous tool at the interface and there is formed a hard armored surface, the improvement which comprises the steps of automatically initiating heating with induction heat induced by the flow of high frequency alternating current

of about 300 kilocycles to about 8 megacycles in said selected portion of the surface of the ferrous tool coated with said pulverulent armor material, automatically continuing said induction heating momentarily to increase the temperature within the skin of the metallic surface of the ferrous tool and to cause heat to flow outwardly from said metallic surface to and through the armor layer to soften the adhesive binder to coat the metallic surface of the ferrous tool with a film to protect the said metallic surface and the pulverulent armor material against oxidation and decarburization and to cause dissipation of the adhesive binder, to convert the fusible flux into a fused state thereby enveloping the underlying metallic surface of the ferrous tool and the outer surface of the armor layer and protecting the ferrous tool and the pulverulent armor material, and to bring the metallic surface of the ferrous tool and the pulverulent armor material to the sweating point thereby enabling the pulverulent armor material to merge into a unitary, refractory metallic armor coating and to bond tenaciously to the metallic surface of the ferrous tool under protection of a film of fused flux on the outer surface of the unitary armor coating, automatically controlling said heating for a short momentary period of time of about a few seconds sufficient to produce a sweating temperature and to cause conversion of said fusible flux into a fused state and to effect bonding of the ferrous tool with said hard, refractory metallic constituent of the armor at the interface between the metallic surface of the ferrous tool and the armor, and discontinuing the induction heating substantially instantaneously after the sweating point has been reached and after the unitary refractory metallic coating of armor material has been bonded to the metallic surface of the ferrous tool and after it has been covered with a film of fused flux while self-cooling is effected by the cooler body of the ferrous tool whereby substantially instantaneous solidification of the hard, refractory metallic armor coating on the ferrous tool and the fused flux over the hard, refractory metallic armor and ferrous tool, whereby armor is formed on the surface of the selected portion of the ferrous tool conforming to the shape thereof and bonded tenaciously and flexibly to the metallic surface of said ferrous tool, and whereby the armor is covered with a fused flux coating.

4. In an armoring method of applying to a selected portion of a surface of a steel article a hard armored surface conforming to the shape of the steel article by a combination of operations including applying to the selected portion of the surface of the steel article an organic adhesive binder having the property of adhesion and holding in place powdered armor material containing a hard refractory metallic matrix alloy, a fusible flux having adhesive properties when fused, and diamond substitute particles composed of at least one carbide selected from the group consisting of the carbides of silicon, tungsten, molybdenum, chromium, tantalum, niobium, vanadium, titanium, zirconium and boron, and subsequently heating the powdered surface to a temperature and for a period of time sufficient to reach the sweating point of the base metal of the steel article whereupon there is a fusion of the matrix of the surface layer and the surface of said steel article at the interface the improvement which comprises the steps of subjecting said underlying surface of said selected portion to intense concentrated heating by means of high frequency induction effected through the skin of the steel article by high frequency alternating electric power of about 300 kilocycles to about 8 megacycles to produce intense heat concentrated on the selected portion of the surface of the steel article and to cause heat to flow outwardly from said metallic surface to and through the armor material, and only momentarily for a few seconds continuing the intense heat concentrated on the selected portion of the surface whereupon the organic adhesive binder is subjected to pyrolysis causing constituents to evaporate, burn and produce reducing

gases and products of combustion and a carbonaceous residue from any residual constituents to protect the steel article, the hard refractory matrix alloy and the diamond substitute particles against oxidation and decarburization while the fusible flux is subjected to fusion to a plastic condition having holding properties and whereupon there is a fusion at the sweating temperature of the hard refractory metallic matrix alloy of the hard armor coating and the surface of said steel article at the interface thereby effecting a fusion of said hard refractory metallic matrix alloy of the armor coating and said metallic surface of said steel article and a merging together in a self-conforming unitary armor layer of substantially uniform thickness with diamond substitute particles tightly fused therein and covered with a fused flux coating enveloping the unitary armor layer.

5. In an armoring method of producing an improved armored steel tool having a thin hard, flexible armor coating which has thinness up to about 0.015 of an inch which has a fusion and interfacial bond located and interposed between the surface of the steel tool and the armor coating and possessing tenaciousness and toughness capable of sustaining intense loads which conforms exactly to the shaping of a regular and irregular underlying surface including horizontal, inclined and vertical surfaces and sharp corners, which has continuity of coverage over the selected coated area to be armored, and which possesses hardness and wear resistance even at high temperatures, by a combination of operations including applying to a specific and selected area of the surface of a steel tool an organic adhesive film and a layer of powdered armoring material comprising a fusible flux having adhesive properties when fused, a hard refractory metallic matrix alloy and diamond substitute particles composed of at least one carbide selected from the group consisting of the carbides of silicon, tungsten, molybdenum, chromium, tantalum, niobium, vanadium, titanium, zirconium and boron, and subsequently heating the coated surface of the steel tool at a temperature and for a period of time sufficient to cause pyrolysis of the organic adhesive, to fuse the flux and to reach the sweating point of the base metal of the steel tool whereupon there is a fusion of the matrix with the surface layer of said steel tool at the interface, the improvement which comprises the steps of turning on high frequency alternating power to subject a specific and selected area of the surface of a steel tool to intense concentrated induction heating by means of high frequency induction effected through the skin of the metallic surface of the steel tool by said high frequency alternating electrical power of at least as high as about 300 kilocycles to produce intense heat concentrated on the specific and selected area of the metallic surface of the steel tool and to cause heat to flow outwardly from the metallic surface to and through the powdered armoring material, and practically instantaneously thereafter turning off said high frequency electric power after the expiration of an extremely short period of time to effect the continuance of the intense induction heat for a few seconds on the surface of the specific and selected surface area whereupon the organic adhesive is subjected to pyrolysis causing constituents to evaporate, burn and produce reducing gases and products of combustion and a carbonaceous residue from any residual constituents to protect the steel tool, the hard refractory matrix alloy and the diamond substitute particles against oxidation and decarburization while the fusible flux is subjected to fusion to a plastic condition having holding properties and whereupon there is a fusion at the sweating temperature of the hard refractory metallic matrix alloy of the hard armor coating and the metallic surface of said hard refractory metallic matrix alloy of the armor coating and the metallic surface of said steel tool and a merging together in a self-conforming unitary armor layer of substantially uniform thinness up to about 0.015 inch with diamond substitute particles tightly fused therein

and with a fused flux coating enveloping the unitary armor layer.

6. In an armoring method of producing an improved armored steel article having a thin, hard, flexible armor coating which has thinness up to about 0.015 of an inch, which has a fusion and interfacial bond located and interposed between the surface of the steel article and the armor coating and possessing tenaciousness and toughness capable of sustaining intense loads, which conforms exactly to the shaping of a regular and irregular underlying surface including horizontal, inclined and vertical surfaces and sharp corners, which has continuity of coverage over the selected coated area to be armored, and which possesses hardness and wear resistance even at high temperatures, by a combination of operations including applying to a surface of a selected area of the metallic base of the steel article a film of liquid organic binder having the property of adhesion, of decomposing as an incident to the method and of a consistency such that it spreads evenly and with a substantially uniform thickness on said surface upon contact therewith, coating the film of organic binder with powdered hard refractory metallic armoring material comprising a powdered hard refractory metallic matrix alloy and powdered diamond substitute particles, and subsequently heating the said selected area of the steel article and the coated surface thereon to a temperature and for a period of time sufficient to reach the sweating point of the base metal of the steel article whereupon the organic binder is subjected to pyrolysis causing volatile constituents to evaporate, burn and produce products of combustion and any residual constituents remaining as a carbonaceous residue whereupon there is a fusion of the hard refractory metallic matrix alloy of the coated surface and the surface of said steel article at the interface, the improvement which comprises the steps of establishing a high frequency electrical induction circuit having a part of said steel article containing said selected area closely coupled therein, causing high frequency alternating electric current of about 300 kilocycles to about 8 megacycles to flow through said induction circuit to concentrate intense electrical inductive heat on the surface skin of the selected area of the coated steel article and to cause heat to flow outwardly from said metallic surface to and through the powdered armor material, controlling said flow of electric current for a momentary period of time of a few seconds to maintain a practically instantaneous heat cycle sufficient to cause pyrolysis of the organic binder and to reach the sweating point of the surface of the selected area of the steel article whereupon there is a fusion of the powdered metallic armor material adhering to the selected area of the coated surface and the steel article at the interface and whereupon the powdered hard refractory metallic armor material and the surface of the selected area of the steel article are tightly bonded together with an interfacial metallic alloy and the diamond substitute particles are tightly fused in the coating layer of armor material, and thereafter substantially instantaneously discontinuing said flow of high frequency alternating electric current whereby further intense heat concentrated on said selected area ceases to be created by induction and whereby substantially instantaneous self-cooling is effected by the body of the steel article.

7. In an armored method of producing an improved armored steel tool having a thin, hard, flexible armor coating which has thinnesses up to about 0.015 of an inch, which has a fusion and interfacial bond located and interposed between the surface of the steel tool and the coating and possessing tenaciousness and toughness capable of sustaining intense loads, which conforms exactly to the shaping of a regular and irregular underlying surface including horizontal, inclined and vertical surfaces and sharp corners, which has continuity of coverage over the selected coated area to be armored, and which possesses hardness and wear resistance even at high temperatures

by a combination of operations including applying to a surface of a specific and selected area of a steel tool a liquid organic adhesive and powdered armor material comprising tungsten carbide, a fusible flux having adhesive properties when fused, and a hard refractory metallic alloy containing tungsten, cobalt and chromium, and subsequently heating the coated surface of the specific and selected area of the steel tool at a temperature and for a period of time sufficient to cause pyrolysis of the organic adhesive, to fuse the flux and to reach the sweating point of the base metal as coated whereupon there is a fusion of the hard refractory metallic alloy of the coated surface and the selected area of the steel tool at the interface, the improvement which comprises the steps of subjecting momentarily the surface of the specific and selected area of a coated steel tool to intense induction heat produced by alternating electric current having a sufficiently high frequency up to about 8 megacycles to increase the temperature practically instantaneously within the skin of the metallic surface of the steel tool to the sweating point and to cause heat to flow outwardly from the metallic surface of the steel tool to and through the coating of powdered armor material, to subject said organic adhesive to pyrolysis, and to subject said fusible flux to fusion to a plastic condition having holding properties, discontinuing said induction heating after a short momentary period of time of a fraction of a minute sufficient to produce a sweating temperature and to cause bonding of the steel tool to the coat of armor having a thinness of about 0.001 of an inch to about 0.015 of an inch and comprising hard refractory metallic alloy containing dispersed particles of tungsten carbide fused therein, and thereafter permitting self cooling of a unitary refractory metallic coat of armor by the cooler body of the steel tool whereby practically instantaneous solidification of the hard refractory metallic armor coat on the steel tool is effected, whereby armor is formed only on the specific and selected area of the steel tool conforming to the contour of the specific and selected area, and whereby the hard refractory metallic alloy of the armor coat and the metallic surface of the steel tool are fused together with an interfacial metallic bonding layer.

8. In an armoring method of applying to a specific and selected portion of a surface of a steel cutting tool a hard armored surface conforming to the shape of the steel cutting tool by a combination of operations including wetting the specific selected portion of a surface of the steel cutting tool to be armored with a liquid binder composition decomposable by heat and of a consistency such that it flows evenly thereon upon contact to provide a film of binder that retains the exact configuration of the surface of the steel cutting tool which it covers, powdering the applied binder with powdered armor material containing a powdered hard refractory metallic matrix material and powdered diamond substitute particles adapted to adhere to the film of binder in a coating layer conforming to the configuration of the underlying surface of the steel cutting tool, and subsequently heating the powdered surface of the specific and selected portion of the steel cutting tool to decompose the binder and to cause fusion of particles of powdered hard refractory metallic matrix material directly upon the underlying surface of the steel cutting tool evenly in a surface-bonded armor, retaining the configuration of the underlying surface, the improvement which comprises the steps of closely coupling a limited part of a steel cutting tool containing a specific and selected portion in an electrical high frequency induction circuit, closing a timing circuit connected with said electrical circuit to cause the flow of very high frequency alternating current up to about 8 megacycles and energizing the circuit to cause the creation of intense induction heat on the surface of the specific and selected portion of the steel cutting tool and to cause the heat to flow outwardly from said metallic surface of the steel cutting tool to and through the powdered armor material,

restricting the intense heat to be concentrated on said specific and selected portion only for a momentary period of time of a fraction of a minute to effect a practically instantaneous heating to the sweating point and a practically instantaneous fusion of the powdered armor material together and to the underlying surface of the specific and selected portion of the steel cutting tool to be armored, and thereafter substantially instantaneously opening said timing circuit to discontinue the flow of very high frequency alternating current in said electrical circuit whereby a steel cutting tool is produced having an exact control of a coated armor adjacent to a cutting edge, a firm controlled penetration of the armor material into the surface of the specific and selected portion of the steel cutting tool to form a tenacious bond between the surface of the steel cutting tool and the coating of hard refractory metallic armor and an effective retention by fusing particles of said diamond substitute within the armor coating and whereby effectiveness of the hard, sharp refractory metallic armor coating is maintained

5

10

15

20

even in service and even when heated in use up to red heat.

**References Cited**

**UNITED STATES PATENTS**

|           |         |               |       |            |
|-----------|---------|---------------|-------|------------|
| 1,591,983 | 6/1924  | Koehnline     | ----- | 117—119.4  |
| 1,726,431 | 8/1929  | Fourment      | ----- | 117—22 X   |
| 1,735,000 | 11/1929 | Dely          | ----- | 117—22 X   |
| 1,998,496 | 4/1935  | Fieldler      | ----- | 117—93.2 X |
| 2,040,767 | 5/1936  | Dudley        | ----- | 117—93.2   |
| 2,223,355 | 12/1940 | Gonser et al. | ----- | 117—52 X   |
| 2,290,338 | 7/1942  | Koehring      | ----- | 117—22 X   |
| 2,360,443 | 10/1944 | Onions        | ----- | 51—295 X   |
| 3,024,128 | 3/1962  | Dawson        | ----- | 117—22 X   |

WILLIAM D. MARTIN, *Primary Examiner.*

PAUL ATTAGUILE, *Assistant Examiner.*

U.S. Cl. X.R.

117—46, 93.1, 93.2; 118—620; 336—62

UNITED STATES PATENT OFFICE  
CERTIFICATE OF CORRECTION

Patent No. 3, 449,146 Dated June 10, 1969  
Inventor(s) Chester H. Dawson

It is certified that error appears in the above-identified patent and that said Letters Patent are hereby corrected as shown below:

1. In Column 6, Line 25, there is an omission of --liquid vehicle, such as water, alcohol, mixtures thereof,-- which should appear after "volatile"; Line 26, "Such an adhesive or binder can contain suitable ingre--" should appear after Line 27; and in Line 28 "such an adhesive or binder can contain suitable ingre--" should be omitted. The corrected sentences in Lines 25 to 29 should read as follows:-

--The temporary adhesive or binder has a volatile liquid vehicle, such as water, alcohol, mixtures thereof, or the like, which can be volatilized and dried readily. Such an adhesive or binder can contain suitable ingredients like shellac or borax.--

2. In Column 10, Line 4, "high" should be --line--.
3. In Column 17, Lines 46 and 47, "(about 0.30" or 0.033")" should read --( about 0.030" or 0.033")--.
4. In Column 19, Line 52, "used" should be --use--; Line 60, "tarmor" should be --armor--; and Line 67 "kuenching" should be --quenching--.
5. In Column 20, Line 33, "or" should be --of--.

SIGNED AND  
SEALED

SEP 1 - 1970

(SEAL)

Attest:

Edward M. Fletcher, Jr.

Attesting Officer

WILLIAM E. SCHUYLER, JR.  
Commissioner of Patents